



US006355403B1

(12) **United States Patent**  
Bourdelais et al.

(10) **Patent No.:** US 6,355,403 B1  
(45) **Date of Patent:** Mar. 12, 2002

(54) **DUPLITIZED REFLECTIVE MEMBERS  
USEFUL FOR ALBUM PAGES**

(75) Inventors: **Robert P. Bourdelais**, Pittsford; **Alphonse D. Camp**, Rochester; **Peter T. Aylward**, Hilton, all of NY (US)

(73) Assignee: **Eastman Kodak Company**, Rochester, NY (US)

(\*) Notice: Subject to any disclaimer, the term of this patent is extended or adjusted under 35 U.S.C. 154(b) by 0 days.

(21) Appl. No.: **09/493,786**

(22) Filed: **Jan. 28, 2000**

(51) **Int. Cl.<sup>7</sup>** ..... G03C 1/46; G03C 1/77; G03C 1/825; G03C 1/795; G03C 1/79

(52) **U.S. Cl.** ..... 430/394; 430/403; 430/432; 430/496; 430/502; 430/510; 430/517; 430/533; 430/536; 430/524; 430/22; 430/952; 430/939

(58) **Field of Search** ..... 430/502, 22, 536, 430/533, 952, 939, 524, 496, 432, 510, 517, 403, 394, 961; 40/768; 281/38; 283/61, 112; 40/79

(56) **References Cited**

U.S. PATENT DOCUMENTS

400,031 A \* 3/1889 Zumwalt ..... 281/38

|             |         |                                 |                              |
|-------------|---------|---------------------------------|------------------------------|
| 4,019,943 A | 4/1977  | Holson                          | ..... 156/227                |
| 4,244,762 A | 1/1981  | Holson                          |                              |
| 4,263,357 A | 4/1981  | Holson                          |                              |
| 4,526,862 A | *       | 7/1985                          | Pelc ..... 430/502           |
| 4,603,428 A | *       | 7/1986                          | Sandrik et al. ..... 430/502 |
| 4,934,739 A | 6/1990  | Stancato                        |                              |
| 4,977,694 A | 12/1990 | Dorman                          |                              |
| 5,242,522 A | 9/1993  | Moir                            |                              |
| 5,791,692 A | 8/1998  | Manico et al. ..... 402/79      |                              |
| 5,866,282 A | 2/1999  | Bourdelais et al. ..... 430/536 |                              |
| 6,017,685 A | 1/2000  | Bourdelais et al. ..... 430/536 |                              |
| 6,020,116 A | 2/2000  | Camp et al. ..... 430/536       |                              |
| 6,027,140 A | 2/2000  | Plutsky                         |                              |
| 6,030,742 A | 2/2000  | Bourdelais et al. ..... 430/536 |                              |
| 6,030,756 A | 2/2000  | Bourdelais et al. ..... 430/536 |                              |
| 6,143,459 A | *       | 11/2000                         | Vizard ..... 430/502         |

\* cited by examiner

*Primary Examiner*—Richard L. Schilling

(74) *Attorney, Agent, or Firm*—Paul A. Leipold

(57) **ABSTRACT**

This invention relates to a photographic element comprising a base having a reflection surface on each side having a spectral transmission of less than 10% and at least one photosensitive silver halide containing layer on each side wherein said photographic element has a speed less than 50 ASA.

**23 Claims, 1 Drawing Sheet**





*FIG. 1*



*FIG. 2*

## DUPLITIZED REFLECTIVE MEMBERS USEFUL FOR ALBUM PAGES

### FIELD OF THE INVENTION

This invention relates to photographic materials. In a preferred form it relates to duplitized photographic reflective images.

### BACKGROUND OF THE INVENTION

In the formation of color paper it is known that the base paper has applied thereto a layer of polymer, typically polyethylene. This layer serves to provide waterproofing to the paper, as well as providing a smooth surface on which the photosensitive layers are formed. The formation of a suitably smooth surface is difficult requiring great care and expense to ensure proper laydown and cooling of the polyethylene layers. The formation of a suitably smooth surface would also improve image quality, as the display material would have more apparent blackness as the reflective properties of the improved base are more specular than the prior materials. As the whites are whiter and the blacks are blacker, there is more range in between and, therefore, contrast is enhanced. It would be desirable if a more reliable and smoother surface could be formed at less expense.

Prior art photographic reflective photographic papers are coated with light sensitive silver halide imaging layers on one side of the paper and thus images only appear on one side of the photographic paper. Typically, the side opposite the imaging layers contains the manufacture brand name and is coated with an antistatic coating. Prior art photographic paper is typically conveyed on the backside during manufacture of the paper and in photographic processing as contact with the numerous rollers and platens in manufacturing and photographic image processing would scratch the imaging layers reducing the quality of the image. Further, photographic printing equipment is currently configured to print only one side of the photographic paper.

Prior art two sided photographs or reflective photographs with images on both sides are accomplished by printing two separate imaging elements containing a light sensitive silver halide coating on one side of the support and adhesively adhering the two developed images back to back after imaging processing. While this process does yield a two-sided photograph that can be utilized for album paging for example, it is expensive and time consuming as thickness of the prior art two-sided photograph is excessive. The thick, two-sided image is difficult to handle, expensive to mail and does not easily fit into photographic albums and frames designed for a single thickness of support material.

It has been proposed in U.S. Pat. No. 5,866,282 Bourdeais et al., to utilize a composite support material with laminated biaxially oriented polyolefin sheets as a photographic imaging material. In U.S. Pat. No. 5,866,282, biaxially oriented polyolefin sheets are extrusion laminated to cellulose paper to create a support for silver halide imaging layers. The biaxially oriented sheets described in U.S. Pat. No. 5,866,282 have a microvoided layer in combination with coextruded layers that contain white pigments. The composite imaging support structure described in U.S. Pat. No. 5,866,282 has been found to be more durable, sharper and brighter than prior art photographic paper imaging supports that use cast melt extruded polyethylene layers coated on cellulose paper.

The continuing thrust towards digital printing of photographic color papers has created the need for a consumer color paper that can work in both negative working optical

and digital exposure equipment. In order for a color paper to correctly print, utilizing a color negative curve shape of the paper is critical. In a digital environment (direct writing) to a photographic paper, the curve shape to a degree can be electromodulated and thus have a greater degree of freedom that the color negative working system. Ideally, a color paper that could substantially maintain tone scale from conventional optical negative working exposure times to sub microsecond digital direct writing exposure times would be preferred. This would enable a photofinishing area to maintain one paper for both digital and optical exposure thereby reducing the need for expensive inventory. Furthermore, digital printing of a page would allow for page composition for album pages.

### PROBLEM TO BE SOLVED BY THE INVENTION

There is a continuing need for silver halide images that can be efficiently printed on both sides of the photographic paper. Further, there is also continuing need for photographic elements that are more durable in use and lighter weight for handling during the formation, imaging, and development process.

### SUMMARY OF THE INVENTION

It is an object of the invention to provide a silver halide image printed on both sides of the support.

It is another object of the invention to overcome disadvantages of prior art and practices.

It is another object to provide photographic elements that are lightweight and thin for ease of handling during formation of the element and its imaging and development.

These and other objects of the invention are accomplished by a photographic element comprising a base having a reflection surface on each side having a spectral transmission of less than 10% and at least one photosensitive silver halide containing layer on each side wherein said photographic element has a speed less than 50 ASA.

### ADVANTAGEOUS EFFECT OF THE INVENTION

The invention provides a photographic element that has images printed on both sides, light in weight for ease of formation, imaging and development but may be easily adhered to a variety of substrates.

### BRIEF DESCRIPTION OF THE DRAWINGS

FIG. 1 is an illustration of the element of the invention exhibiting a duplitized photographic image suitable for an album page.

Illustrated in FIG. 2 is a top view of a duplitized silver halide album page that has been composed and contains punched holes for insertion into a ringed album binder.

### DETAILED DESCRIPTION OF THE INVENTION

The invention has numerous advantages over prior photographic elements. The two-sided photograph of the invention allows for high quality silver halide reflective images to be printed on the front side and the backside of a photograph. A two sided photograph has allows a 50% reduction in storage space for images as a single thickness of photographic contains two images. Further, several cost reductions are now possible as mailing and shipping cost have

been reduced by 50% and the amount of reflective support material is also reduced by 50% since one thickness of reflective support material yields two images. By binding the two sided print, photographic books and albums are possible and are thin because the support thickness has been reduced by 50% compared to the prior art technique to adhering two one sided images back to back.

The two-sided image may also be utilized to write critical information on the backside of the image. Personal information such as time, date and location of a photograph can now be silver halide printed on the backside of the two-sided image allowing for each photograph to be personalized. The two-sided image can also be utilized for localized advertisement on the backside of the image. Examples of advertisements printed on the backside include continuity coupons, branding by the photographic processing lab and promotional contests. The invention also provides an opportunity to utilize duplitzied silver halide printing technology to provide reflective images on both sides of a tough support. The duplitzied tough support materials can be used for applications that require images and printing on both sides of a durable support. Examples of a durable silver halide duplitzied printing material include identification cards, collection cards such as baseball cards, greeting cards and photographic licenses.

The support material utilized in the invention allows for the simultaneous printing of both sides of the image without suffering from unwanted light exposure from one side to the other side of the light sensitive imaging layers. Digital printing of the image either through a digital working silver halide printing system or through ink jet printing allows information such as exposure information, date and time of exposure and subject matter to be attached to the image easily and without fear of loss of this critical information. Further, digital printing, especially in the silver halide imaging layers allows for improved image sharpness and dye hue of the color couplers utilized in this invention. These and other advantages will be apparent from the detailed description below.

The term as used herein, "transparent" means the ability to pass radiation without significant deviation or absorption. For this invention, "transparent" material is defined as a material that has a spectral transmission greater than 90%. For a photographic element, spectral transmission is the ratio of the transmitted power to the incident power and is expressed as a percentage as follows;  $T_{RGB}=10^{-D}*100$  where D is the average of the red, green and blue Status A transmission density response measured by an X-Rite model 310 (or comparable) photographic transmission densitometer. For this invention, "reflective" print material or base or polymer base is defined as a material that has a spectral transmission of 10% or less.

For the photographic element of this invention the light sensitive silver halide emulsion layer is coated onto both sides of the reflective base. This duplitzied photographic element can then be printed with images on both sides using conventional silver halide exposure technology or digital exposure technology and processed using traditional photographic chemistry. This method for creating a two sided print is preferred as the cost of the base material is reduced by 50% as two images are supported by only one reflective base element compared to prior art two sided images which comprise two separate images adhesively adhered after image development. Further, by applying the light sensitive silver halide imaging layers on both sides of the support, the costly and difficult task of adhering to images back to back is avoided.

The speed of the light sensitive silver halide imaging layers is preferably less than 50 ASA. Reflective paper silver halide emulsion speed is determined by the following formula:

$$5 \quad \text{Emulsion Speed} = (1000/H_{0.6})$$

Where  $H_{0.6}$  is the exposure (lux-second) required to produce a density 0.6 above base plus fog density. A speed of less than 50 ASA is preferred, as faster light sensitive silver halide imaging layers have been shown to suffer from unwanted exposure of the opposite side as one side is being printed with exposure light energy.

The spectral light transmission of the base material is preferably less than 10%. A spectral light transmission of less than 10% is required to prevent exposure light energy from traveling though the base material and creating an unwanted exposure of the opposite side. The most preferred spectral transmission of the reflecting base is less than 2% as the exposure light energy does not significantly impact the quality of the image on the opposite side.

The duplitzied reflection paper of the invention can be used to create album pages by exposing both sides of the duplitzied support; developing the image and punching index holes for the paper. The album page can also be post

25 process laminated with a protective polymer sheet to provide image protection while in the consumer photographic album. When digital printing methods are utilized to print images, both sides of the album page can be composed allowing the images to be grouped in a meaningful way.

30 Further, digital composition of the duplitzied support can be used to print boarders or other information in the margin areas of the composed page.

By utilizing digital printing methods such as lasers and CRT printers, the second exposure for the two sided photographic member can also be utilized for the printing of the same image that has been corrected by a image printing algorithm to provide the consumer with two different printing settings. The second exposure can also be utilized to provide stock photographic images that are consistent with 40 the theme of the photographic subject. For example, the subject matter if the consumer images comprises nature scenes then stock photographic images of nature scenes could be printed on the opposite side to add to the viewing pleasure of the consumer.

45 Because light sensitive silver halide layers are applied to both the top and bottom sides of the support, great care must be taken during image exposure so that the exposure light energy from one side of the imaging element does not expose the light sensitive layers of the opposite side. To 50 reduce the undesirable exposure of the opposite image, the reflective support of the invention preferably contains an opacifying layer. The opacifying layer in the reflective support blocks the exposure light energy from reaching the opposite side, thereby reducing unwanted exposure of the opposite side. Preferred support opacifying layers are metallic foils and carbon black or black dyes dispersed in a polymer layer. Both the metallic foil and the layer of carbon black or black dyes in a polymer layer have been shown to provide spectral transmission of less than 2%. The opacifying 55 layer may be located in any layer between the two light sensitive imaging layers. Preferably, the opacifying layer is in a layer that does not interfere with the image. An example is the location of a metallic foil layer below the microvoided layer of a preferred biaxially oriented sheet. The gas containing voided layer between the metallic foil layer and the imaging layers provides sufficient opacity so that the image 60 quality is maintained.

Another unique feature of this invention is the addition of an antihalation layer to the light sensitive bottom imaging layer. The antihalation layer prevents unwanted exposure of the opposite side as light is absorbed in the antihalation layer during exposure. During exposure, the antihalation layer absorbs light energy that could cause unwanted exposure of the opposite side. During image development, the antihalation layer is rendered transparent, so that the bottom silver halide formed image can be viewed in reflection space.

A considerable amount of light may be diffusely transmitted by the emulsion and strike the back surface of the support. This light is partially or totally reflected back to the emulsion and reexposed it at a considerable distance from the initial point of entry. This effect is called halation because it causes the appearance of halos around images of bright objects. Further, a transparent support also may pipe light. Halation can be greatly reduced or eliminated by absorbing the light transmitted by the emulsion or piped by the support. Three methods of providing halation protection are (1) coating an antihalation undercoat which is either dye gelatin or gelatin containing gray silver between the emulsion and the support, (2) coating the emulsion on a support that contains either dye or pigments, and (3) coating the emulsion on a transparent support that has a dye or pigment a layer coated on the back. The absorbing material contained in the antihalation undercoat or antihalation backing is removed by processing chemicals when the photographic element is processed. In the instant invention, it is preferred that the antihalation layer be formed of gray silver which is coated on the side furthest from the top and removed during processing. By coating furthest from the top on the back surface, the antihalation layer is easily removed, as well as allowing exposure of the duplitzied material from only one side. If the material is not duplitzied, the gray silver could be coated between the support and the top emulsion layers where it would be most effective. The problem of halation is minimized by coherent collimated light beam exposure, although improvement is obtained by utilization of an antihalation layer even with collimated light beam exposure.

Because the duplitzied silver halide imaging material must be transported through manufacturing and imaging processing, one of the light sensitive imaging layers will contact transport rollers and metal guiding plates. The use of a material that provides stand off of the light sensitive silver halide imaging layers from the surfaces of transport rollers is preferred. The protective overcoat for the light sensitive silver halide emulsions preferably contains a matte bead. The matte bead is required to create a separation between the emulsion layers when the imaging element is wound in rolls. The matte bead creates a separation between the duplitzied imaging layers that prevents roll blocking as gelatin layers tend to adhere especially in the presence of moisture. The matte beads also allow for a light sensitive silver halide imaging layer to be transported through manufacturing and photographic processing equipment without scratching the imaging layers. Preferred matte beads are small polymer beads with a mean particle size less than 25 micrometers. A preferred matte bead is methylene methacrylate.

The duplitzied image is preferably formed by exposing one side of the invention to light energy and then exposing the second side. The imaging layers on each side of the base preferably are exposed substantially simultaneously. Simultaneous exposure is preferred as the productivity of the imaging printing process is improved and the need for imaging material rotation in the printing equipment is avoided.

After image printing and development, the duplitzied imaging material is preferably has applied to the surface a

protective polymer. A protective polymer is preferred as it protects the developed image layers from dirt, scratches, fingerprints and water. The protective polymer also eliminates the need for consumers to place developed images in protective sleeves. Preferred polymers include aqueous polyester, latex, acrylics and styrene butadiene. The protective polymer may also be a preformed polymer sheet that is oriented for strength. Preferred oriented polymers include polyolefin, polyester and nylon.

10 After the image is developed, holes are preferably punched along the perimeter to allow for easy placement in a photographic album. For example, a three hole punch along one side of the imaged duplitzied image material will allow for easy storage in typical photographic albums that 15 contain a three keeper rings.

The reflective base material of the invention preferably is white, reflecting and free of pinholes. A base material with a tear resistance of greater than 150 N is preferred as the strength of the materials allows the use of punched holes in 20 the base material for use in photographic albums with keeper rings without the need for expensive grommets for reinforcement. It has been found that bases with a tear resistance less than 125 N frequently fracture in a photographic album application.

25 A base substantially free of pinholes avoids the unwanted exposure of the opposite side during the exposure step of the imaging process as exposure light energy can travel through pinholes in the base material.

The base material of the invention is preferably has a 30 stiffness greater than 100 millinewtons. A stiffness of 100 millinewtons is required for web transport through photographic processing equipment that is typically edge guided. A base with a stiffness greater than 100 millinewtons is also required to create a high quality album page as stiffness less 35 than 80 millinewtons would fold over and crease, reducing the quality of the image. A base stiffness less than 350 millinewtons is preferred as additional stiffness would not significantly add to the quality of a two-sided print material. Further, a stiffness of 400 millinewtons is difficult to punch and chop in photographic processing equipment.

40 The base material of the invention preferably has an L\* or lightness greater than 93.5. It has been found that L\* greater than 93.5 provide excellent whites and improve the contrast range of the image. Further, an L\* greater than 93.5 allows 45 for an improved dye gamut compared to photographic bases with an L\* less than 92.0.

Illustrated in FIG. 1 is a cross section of a duplitzied silver halide album page. Imaging base 10 has applied thereto an upper developed silver halide imaging layer 12 and a lower 50 developed silver halide imaging layer 14. The upper imaged layer 12 has a polymer sheet 16 adhesively adhered to 12 for protection of the developed imaged layer. The lower imaged layer 14 has a polymer sheet 18 adhesively adhered to 14 for protection of the developed image layer. Polymer sheet 16 and 18 were adhesively adhered to imaged layers 12 and 14 55 after imaging processing.

Illustrated in FIG. 2 is a top view of a duplitzied silver halide album page that has been composed and contains punched holes for insertion into a ringed album binder. The 60 duplitzied imaged element 20 contains four images 22, 24, 26 and 28 that have been arranged and digitally printed on 20 and contain spaces between the images 22, 24, 26 and 28. Holes 30, 32 and 34 are then punched into the imaged duplitzied silver halide album page for insertion into a 65 ringed binder.

The preferred base materials utilized in the invention are base materials that comprise a paper core and base materials

that contain a polymer core. In the case of a paper core a polymer extrusion coating or adhesive lamination of polymers is required to provide water resistance to the paper as the light sensitive silver halide imaging layers are developed in wet chemistry, typically RA-4 process chemistry. The paper core of the invention needs to be smooth, strong and not react with the light sensitive silver halide imaging layers. Preferred photographic grade cellulose papers are disclosed in U.S. Pat. No. 5,288,690. To form a quality image the paper should have a surface roughness average less than 0.44 micrometers, have a density of between 1.05 and 1.20 grams/cc and utilize cellulose fibers that have an average length between 0.40 and 0.58 mm.

Because the cellulose paper base of the invention does not have the desired strength and imaging processing solution hold out characteristics to withstand wet imaging processing, the cellulose paper core must be protected. The preferred methods for protecting the cellulose paper are extrusion coating of a polymer on the paper surface and adhesive lamination of an oriented polymer sheet. The reflective support of the present invention preferably includes a resin layer with a stabilizing amount of hindered amine extruded on the top side of the imaging layer substrate. Hindered amine light stabilizers (HALS) originate from 2,2,6,6-tertramethylpiperidine. The hindered amine should be added to the polymer layer at about 0.01-5% by weight of said resin layer in order to provide resistance to polymer degradation upon exposure to UV light. The preferred amount is at about 0.05-3% by weight. This provides excellent polymer stability and resistance to cracking and yellowing while keeping the expense of the hindered amine to a minimum. Examples of suitable hindered amines with molecular weights of less than 2300 are Bis(2,2,6,6-tertramethyl-4-piperidinyl)sebacate; Bis(1,2,2,6,6-pentamethyl-4-piperidinyl)sebacate and Bis(1,2,2,6,6-pentamethyl-4-piperidinyl)2-n-butyl-(3,5-di-tert-butylhydroxybenzyl)malonate.

Preferred polymers for the melt extruded waterproof layer include polyethylene, polypropylene, polymethylpentene, polystyrene, polybutylene, and mixtures thereof. Polyolefin copolymers, including copolymers of polyethylene, propylene and ethylene such as hexene, butene, and octene are also useful. Polyethylene is most preferred, as it is low in cost and has desirable coating properties. As polyethylene, usable are high-density polyethylene, low-density polyethylene, linear low density polyethylene, and polyethylene blends. Other suitable polymers include polyesters produced from aromatic, aliphatic or cycloaliphatic dicarboxylic acids of 4-20 carbon atoms and aliphatic or alicyclic glycols having from 2-24 carbon atoms. Examples of suitable dicarboxylic acids include terephthalic, isophthalic, phthalic, naphthalene dicarboxylic acid, succinic, glutaric, adipic, azelaic, sebacic, fumaric, maleic, itaconic, 1,4-cyclohexanedicarboxylic, sodiosulfoisophthalic and mixtures thereof. Examples of suitable glycols include ethylene glycol, propylene glycol, butanediol, pentanediol, hexanediol, 1,4-cyclohexanediethanol, diethylene glycol, other polyethylene glycols and mixtures thereof. Other polymers are matrix polyesters having repeat units from terephthalic acid or naphthalene dicarboxylic acid and at least one glycol selected from ethylene glycol, 1,4-butanediol and 1,4-cyclohexanediethanol such as poly(ethylene terephthalate), which may be modified by small amounts of other monomers. Other suitable polyesters include liquid crystal copolymers formed by the inclusion of suitable amount of a co-acid component such as stilbene dicarboxylic acid. Examples of such liquid crystal copolymers are

those disclosed in U.S. Pat. Nos. 4,420,607; 4,459,402; and 4,468,510. Useful polyamides include nylon 6, nylon 66, and mixtures thereof. Copolymers of polyamides are also suitable continuous phase polymers. An example of a useful polycarbonate is bisphenol-A polycarbonate. Cellulosic esters suitable for use as the continuous phase polymer of the composite sheets include cellulose nitrate, cellulose triacetate, cellulose diacetate, cellulose acetate propionate, cellulose acetate butyrate, and mixtures or copolymers thereof. Useful polyvinyl resins include polyvinyl chloride, poly(vinyl acetal), and mixtures thereof. Copolymers of vinyl resins can also be utilized.

Any suitable white pigment may be incorporated in the melt extruded polyolefin waterproof layer, such as, for example, zinc oxide, zinc sulfide, zirconium dioxide, white lead, lead sulfate, lead chloride, lead aluminate, lead phthalate, antimony trioxide, white bismuth, tin oxide, white manganese, white tungsten, and combinations thereof. The preferred pigment is titanium dioxide because of its high refractive index, which gives excellent optical properties at a reasonable cost. The pigment is used in any form that is conveniently dispersed within the polyolefin. The preferred pigment is anatase titanium dioxide. The most preferred pigment is rutile titanium dioxide because it has the highest refractive index at the lowest cost. The average pigment diameter of the rutile  $TiO_2$  is most preferably in the range of 0.1 to 0.26  $\mu m$ . The pigments that are greater than 0.26  $\mu m$  are too yellow for an imaging element application and the pigments that are less than 0.1  $\mu m$  are not sufficiently opaque when dispersed in polymers. Preferably, the white pigment should be employed in the range of from about 10 to about 50 percent by weight, based on the total weight of the polyolefin coating. Below 10 percent  $TiO_2$ , the imaging system will not be sufficiently opaque and will have inferior optical properties. Above 50 percent  $TiO_2$ , the polymer blend is not manufacturable. The surface of the  $TiO_2$  can be treated with an inorganic compounds such as aluminum hydroxide, alumina with a fluoride compound or fluoride ions, silica with a fluoride compound or fluoride ion, silicon hydroxide, silicon dioxide, boron oxide, boria-modified silica (as described in U.S. Pat. No. 4,781,761), phosphates, zinc oxide,  $ZrO_2$ , etc. and with organic treatments such as polyhydric alcohol, polyhydric amine, metal soap, alkyl titanate, polysiloxanes, silanes, etc. The organic and inorganic  $TiO_2$  treatments can be used alone or in any combination. The amount of the surface treating agents is preferably in the range of 0.2 to 2.0% for the inorganic treatment and 0.1 to 1% for the organic treatment, relative to the weight of the weight of the titanium dioxide. At these levels of treatment the  $TiO_2$  disperses well in the polymer and does not interfere with the manufacture of the imaging support.

The melt extruded polyolefin waterproof polymer, hindered amine light stabilizer, and the  $TiO_2$  are mixed with each other in the presence of a dispersing agent. Examples of dispersing agents are metal salts of higher fatty acids such as sodium palmitate, sodium stearate, calcium palmitate, sodium laurate, calcium stearate, aluminum stearate, magnesium stearate, zirconium octylate, zinc stearate, etc, higher fatty acids, and higher fatty amide. The preferred dispersing agent is sodium stearate and the most preferred dispersing agent is zinc stearate. Both of these dispersing agents give superior whiteness to the resin-coated layer.

For photographic use, a white base with a slight bluish tint is preferred. The layers of the melt extruded polyolefin waterproof layer coating preferably contain colorants such as a bluing agent and magenta or red pigment. Applicable bluing agents include commonly known ultramarine blue,

cobalt blue, oxide cobalt phosphate, quinacridone pigments, and a mixture thereof. Applicable red or magenta colorants are quinacridones and ultramarines.

The melt extruded polyolefin waterproof layer may also include a fluorescing agent, which absorbs energy in the UV region and emit light largely in the blue region. Any of the optical brightener referred to in U.S. Pat. No. 3,260,715 or a combination thereof would be beneficial.

The hindered amine light stabilizer,  $TiO_2$ , colorants, slip agents, optical brightener, and antioxidant are incorporated either together or separately with the polymer using a continuous or Banbury mixer. A concentrate of the additives in the form of a pellet is typically made. The concentration of the rutile pigment can be from 20% to 80% by weight of the masterbatch. The master batch is then 15 adequately diluted for use with the resin.

To form the melt extruded polyolefin waterproof layer according to the present invention, the pellet containing the pigment and other additives is subjected to hot-melt coating onto a running support of paper or synthetic paper. If desired, the pellet is diluted with a polymer prior to hot melt coating. For a single layer coating the resin layer may be formed by lamination. The die is not limited to any specific type and may be any one of the common dies such as a T-slot or coat hanger die. An exit orifice temperature in heat melt extrusion of the melt extruded polyolefin waterproof layer ranges from 250 to 370° C. Further, before coating the support with resin, the support may be treated with an activating treatment such as corona discharge, flame, ozone, plasma, or glow discharge.

At least two melt extruded polymer layers applied to the top or bottom side of the tough paper is preferred. Two or more layers are preferred at different polymers systems can be used to improve image whiteness by using a higher weight percent of white pigments or by the use of a less expensive polymer located next to the base paper. The preferred method for melt extruding 2 or more layers is melt coextrusion from a slit die. Coextrusion is a process that provides for more than one extruder to simultaneously pump molten polymer out through a die in simultaneous yet discrete layers. This is accomplished typically through the use of a multimanifold feedblock which serves to collect the hot polymer keeping the layers separated until the entrance to the die where the discrete layers are pushed out between the sheet and paper to adhere them together. Coextrusion lamination is typically carried out by bringing together the biaxially oriented sheet and the base paper with application of the bonding agent between the base paper and the biaxially oriented sheet followed by their being pressed together in a nip such as between two rollers.

The thickness of the melt extruded polyolefin waterproof layer which is applied to a base paper of the reflective support used in the present invention at a side for imaging, is preferably in the range of 5 to 100  $\mu m$  and most preferably in the range of 10 to 50  $\mu m$ . The surface of the waterproof resin coating at the imaging side may be a glossy, fine, silk, grain, or matte surface. On the surface of the water-proof coating on the backside which is not coated with an imaging element may also be glossy, fine, silk, or matte surface. The preferred water-proof surface for the backside away from the imaging element is matte.

A melt extruded layer of polyester applied to the base paper is preferred as the melt extruded polyester provides mechanical toughness and tear resistance compared to typical melt extruded polyethylene. Further, a melt extruded layer of polyester is preferred as the weight percent of white pigment contained in polyester can be significantly

increased compared to the weight percent of white pigment in polyolefin thus improving the whiteness of a polyester melt extruded imaging support material. Such polyester melt extruded layers are well known, widely used and typically prepared from high molecular weight polyesters prepared by condensing a dihydric alcohol with a dibasic saturated fatty acid or derivative thereof.

Suitable dihydric alcohols for use in preparing such polyesters are well known in the art and include any glycol 10 wherein the hydroxyl groups are on the terminal carbon atom and contain from two to twelve carbon atoms such as, for example, ethylene glycol, propylene glycol, trimethylene glycol, hexamethylene glycol, decamethylene glycol, dodecamethylene glycol, 1,4-cyclohexane, dimethanol, and the like.

Suitable dibasic acids useful for the preparation of polyesters include those containing from two to sixteen carbon atoms such as adipic acid, sebacic acid, isophthalic acid, terephthalic acid, and the like. Alkyl esters of acids such as 20 those listed above can also be employed. Other alcohols and acids as well as polyesters prepared therefrom and the preparation of the polyesters are described in U.S. Pat. Nos. 2,720,503 and 2,901,466. Polyethylene terephthalate is preferred.

25 Melt extrusion of the polyester layer to the base paper is preferred. The thickness of the polyester layer is preferably from 5 to 100 micrometers. Below 4 micrometers the polyester layer begins to loose waterproof properties needed to survive a wet image development process. Above 110 30 micrometers, the melt extruded polyester layer becomes brittle and will show undesirable cracks under the image layers.

In addition to melt cast extrusion coating of polymers on 35 to the paper base core, the paper base of the invention preferably is laminated with oriented polymer sheet. Oriented polymer sheet have been shown to improve the tear resistance of the base material, reduce the curl of the image element and are generally capable of providing improved image sharpness and brightness compared to melt cast 40 polymers. Examples of preferred biaxially oriented polymer sheet are disclosed in U.S. Pat. Nos. 5,866,282; 5,853,965; 5,874,205; 5,888,643; 5,888,683; 5,902,720 and 5,935,690. Further, the biaxially oriented sheets laminated to cellulose 45 paper, which are high in strength, have tear resistance greater than 150 N allowing for photographic album hole punches to be made without the need for expensive grommets.

While the paper base core of the invention does provide 50 an acceptable, low cost image, the image quality and durability of the duplitized imaging element can further be improved by utilizing a polymer support material. Preferred polymer support materials include polyester, microvoided polyester and polyolefin. Examples of preferred polymer 55 image support bases are disclosed in U.S. Pat. Nos. 4,912,333; 4,999,312 and 5,055,371. Further, the biaxially oriented polyester, which are high in strength, have tear resistance greater than 150 N allowing for photographic album 60 hole punches to be made without the need for expensive grommets. Tear resistance for the photographic elements is the moment of force required to start a tear along an edge of the photographic element. The tear resistance test used was originally proposed by G. G. Gray and K. G. Dash, Tappi Journal 57, pages 167-170 published in 1974. The tear resistance for the photographic elements is determined by the tensile strength and the stretch of the photographic 65 element. A 15 mm $\times$ 25 mm sample is looped around a metal cylinder with a 2.5 cm diameter. The two ends of the sample

are clamped by an Instron tensile tester. A load is applied to the sample at a rate of 2.5 cm per minute until a tear is observed at which time the load, expressed in N, is recorded.

White pigment weight percents of between 24% and 60% have been demonstrated in oriented polyester further improving the opacity of the base material compared to melt cast or oriented polyolefin.

An preferred example of a base material that can be utilized for a duplitized photographic print material suitable for an album page is as follows where the light sensitive silver halide imaging layers are applied to the oriented polyethylene skin layers on both sides:

Oriented polyethylene skin layer

Microvoided polypropylene

Oriented polypropylene with  $TiO_2$

Aluminum foil layer

Melt extruded EMA

Cellulose paper

Melt extruded EMA

Oriented polypropylene with  $TiO_2$

Voided polypropylene

Oriented polyethylene skin layer

Disclosed below is a suitable flesh tone optimized light sensitive silver halide emulsion capable of accurately reproducing flesh tones. This invention is directed to a silver halide depth image of excellent performance when exposed by either an electronic printing method or a conventional optical printing method. An electronic printing method comprises subjecting a radiation sensitive silver halide emulsion layer of a recording element to actinic radiation of at least  $10^{-4}$  ergs/cm<sup>2</sup> for up to 100  $\mu$ seconds duration in a pixel-by-pixel mode wherein the silver halide emulsion layer is comprised of silver halide grains as described above. A conventional optical printing method comprises subjecting a radiation sensitive silver halide emulsion layer of a recording element to actinic radiation of at least  $10^{-4}$  ergs/cm<sup>2</sup> for  $10^{-3}$  to 300 seconds in an imagewise mode wherein the silver halide emulsion layer is comprised of silver halide grains as described above.

This invention in a preferred embodiment utilizes a radiation-sensitive emulsion comprised of silver halide grains (a) containing greater than 50 mole percent chloride, based on silver, (b) having greater than 50 percent of their surface area provided by {100} crystal faces, and (c) having a central portion accounting for from 95 to 99 percent of total silver and containing two dopants selected to satisfy each of the following class requirements: (i) a hexacoordination metal complex which satisfies the formula



wherein n is zero, -1, -2, -3 or -4; M is a filled frontier orbital polyvalent metal ion, other than iridium; and  $L_6$  represents bridging ligands which can be independently selected, provided that least four of the ligands are anionic ligands, and at least one of the ligands is a cyano ligand or a ligand more electronegative than a cyano ligand; and (ii) an iridium coordination complex containing a thiazole or substituted thiazole ligand.

It has been discovered quite surprisingly that the combination of dopants (i) and (ii) provides greater reduction in reciprocity law failure than can be achieved with either dopant alone. Further, unexpectedly, the combination of dopants (i) and (ii) achieve reductions in reciprocity law failure beyond the simple additive sum achieved when employing either dopant class by itself. It has not been reported or suggested prior to this invention that the combination of dopants (i) and (ii) provides greater reduction in reciprocity law failure, particularly for high intensity and short duration exposures. The combination of dopants (i)

and (ii) further unexpectedly achieves high intensity reciprocity with iridium at relatively low levels, and both high and low intensity reciprocity improvements even while using conventional gelatino-peptizer (e.g., other than low methionine gelatino-peptizer).

In a preferred practical application, the advantages of the invention can be transformed into increased throughput of digital substantially artifact-free color print images while exposing each pixel sequentially in synchronism with the digital data from an image processor.

In one embodiment, the present invention represents an improvement on the electronic printing method. Specifically, this invention in one embodiment is directed to an electronic printing method which comprises subjecting a radiation sensitive silver halide emulsion layer of a recording element to actinic radiation of at least  $10^{-4}$  ergs/cm<sup>2</sup> for up to 100  $\mu$ seconds duration in a pixel-by-pixel mode. The present invention realizes an improvement in reciprocity failure by selection of the radiation sensitive silver halide emulsion layer. While certain embodiments of the invention are specifically directed towards electronic printing, use of the emulsions and elements of the invention is not limited to such specific embodiment, and it is specifically contemplated that the emulsions and elements of the invention are also well suited for conventional optical printing.

It has been unexpectedly discovered that significantly improved reciprocity performance can be obtained for silver halide grains (a) containing greater than 50 mole percent chloride, based on silver, and (b) having greater than 50 percent of their surface area provided by {100} crystal faces by employing a hexacoordination complex dopant of class (i) in combination with an iridium complex dopant comprising a thiazole or substituted thiazole ligand. The reciprocity improvement is obtained for silver halide grains employing conventional gelatino-peptizer, unlike the contrast improvement described for the combination of dopants set forth in U.S. Pat. Nos. 5,783,373 and 5,783,378, which requires the use of low methionine gelatino-peptizers as discussed therein, and which states it is preferable to limit the concentration of any gelatino-peptizer with a methionine level of greater than 30 micromoles per gram to a concentration of less than 1 percent of the total peptizer employed. Accordingly, in specific embodiments of the invention, it is specifically contemplated to use significant levels (i.e., greater than 1 weight percent of total peptizer) of conventional gelatin (e.g., gelatin having at least 30 micromoles of methionine per gram) as a gelatino-peptizer for the silver halide grains of the emulsions of the invention. In preferred embodiments of the invention, gelatino-peptizer is employed which comprises at least 50 weight percent of gelatin containing at least 30 micromoles of methionine per gram, as it is frequently desirable to limit the level of oxidized low methionine gelatin which may be used for cost and certain performance reasons.

In a specific, preferred form of the invention it is contemplated to employ a class (i) hexacoordination complex dopant satisfying the formula:



where

n is zero, -1, -2, -3 or -4;

M is a filled frontier orbital polyvalent metal ion, other than iridium, preferably  $Fe^{+2}$ ,  $Ru^{+2}$ ,  $Os^{+2}$ ,  $Co^{+3}$ ,  $Rh^{+3}$ ,  $Pd^{+4}$  or  $Pt^{+4}$ , more prefer iron, ruthenium or osmium ion, and most preferably a ruthenium ion;

$L_6$  represents six bridging ligands which can be independently selected, provided that least four of the ligands are anionic ligands and at least one (preferably at least 3 and optimally at least 4) of the ligands is a cyano ligand or a ligand more electronegative than a cyano ligand. Any

remaining ligands can be selected from among various other bridging ligands, including aquo ligands, halide ligands (specifically, fluoride, chloride, bromide and iodide), cyanate ligands, thiocyanate ligands, selenocyanate ligands, tellurocyanate ligands, and azide ligands. Hexacoordinated transition metal complexes of class (i) which include six cyano ligands are specifically preferred.

Illustrations of specifically contemplated class (i) hexacoordination complexes for inclusion in the high chloride grains are provided by Olm et al U.S. Pat. No. 5,503,970 and Daubendiek et al U.S. Pat. Nos. 5,494,789 and 5,503,971, and Keevert et al U.S. Pat. No. 4,945,035, as well as Murakami et al Japanese Patent Application Hei-2[1990]-249588, and Research Disclosure Item 36736. Useful neutral and anionic organic ligands for class (ii) dopant hexacoordination complexes are disclosed by Olm et al U.S. Pat. No. 5,360,712 and Kuromoto et al U.S. Pat. No. 5,462,849.

Class (i) dopant is preferably introduced into the high chloride grains after at least 50 (most preferably 75 and optimally 80) percent of the silver has been precipitated, but before precipitation of the central portion of the grains has been completed. Preferably class (i) dopant is introduced before 98 (most preferably 95 and optimally 90) percent of the silver has been precipitated. Stated in terms of the fully precipitated grain structure, class (i) dopant is preferably present in an interior shell region that surrounds at least 50 (most preferably 75 and optimally 80) percent of the silver and, with the more centrally located silver, accounts the entire central portion (99 percent of the silver), most preferably accounts for 95 percent, and optimally accounts for 90 percent of the silver halide forming the high chloride grains. The class (i) dopant can be distributed throughout the interior shell region delimited above or can be added as one or more bands within the interior shell region.

Class (i) dopant can be employed in any conventional useful concentration. A preferred concentration range is from  $10^{-8}$  to  $10^{-3}$  mole per silver mole, most preferably from  $10^{-6}$  to  $5 \times 10^{-4}$  mole per silver mole.

The following are specific illustrations of class (i) dopants:

- (i-1)  $[\text{Fe}(\text{CN})_6]^{-4}$
- (i-2)  $[\text{Ru}(\text{CN})_6]^{-4}$
- (i-3)  $[\text{Os}(\text{CN})_6]^{-4}$
- (i-4)  $[\text{Rh}(\text{CN})_6]^{-3}$
- (i-5)  $[\text{Co}(\text{CN})_6]^{-3}$
- (i-6)  $[\text{Fe}(\text{pyrazine})(\text{CN})_5]^{-4}$
- (i-7)  $[\text{RuCl}(\text{CN})_5]^{-4}$
- (i-8)  $[\text{OsBr}(\text{CN})_5]^{-4}$
- (i-9)  $[\text{RhF}(\text{CN})_5]^{-3}$
- (i-10)  $[\text{In}(\text{NCS})_6]^{-3}$
- (i-11)  $[\text{FeCO}(\text{CN})_5]^{-3}$
- (i-12)  $[\text{RuF}_2(\text{CN})_4]^{-4}$
- (i-13)  $[\text{OsCl}_2(\text{CN})_4]^{-4}$
- (i-14)  $[\text{RhL}_2(\text{CN})_4]^{-3}$
- (i-15)  $[\text{Ga}(\text{NCS})_6]^{-3}$
- (i-16)  $[\text{Ru}(\text{CN})_5(\text{OCN})]^{-4}$
- (i-17)  $[\text{Ru}(\text{CN})_5(\text{N}_3)]^{-4}$
- (i-18)  $[\text{Os}(\text{CN})_5(\text{SCN})]^{-4}$
- (i-19)  $[\text{Rh}(\text{CN})_5(\text{SeCN})]^{-3}$
- (i-20)  $[\text{Os}(\text{CN})\text{Cl}_5]^{-4}$
- (i-21)  $[\text{Fe}(\text{CN})_3\text{Cl}_3]^{-3}$
- (i-22)  $[\text{Ru}(\text{CO})_2(\text{CN})_4]^{-1}$

When the class (i) dopants have a net negative charge, it is appreciated that they are associated with a counter ion when added to the reaction vessel during precipitation. The counter ion is of little importance, since it is ionically dissociated from the dopant in solution and is not incorporated within the grain. Common counter ions known to be fully compatible with silver chloride precipitation, such as ammonium and alkali metal ions, are contemplated. It is

noted that the same comments apply to class (ii) dopants, otherwise described below.

The class (ii) dopant is an iridium coordination complex containing at least one thiazole or substituted thiazole ligand. Careful scientific investigations have revealed Group VIII hexahalo coordination complexes to create deep electron traps, as illustrated R. S. Eachus, R. E. Graves and M. T. Olm *J. Chem. Phys.*, Vol. 69, pp. 4580-7 (1978) and *Physica Status Solidi A*, Vol. 57, 429-37 (1980) and R. S. Eachus and M. T. Olm *Annu. Rep. Prog. Chem. Sect. C. Phys. Chem.*, Vol. 83, 3, pp. 3-48 (1986). The class (ii) dopants employed in the practice of this invention are believed to create such deep electron traps. The thiazole ligands may be substituted with any photographically acceptable substituent which does not prevent incorporation of the dopant into the silver halide grain. Exemplary substituents include lower alkyl (e.g., alkyl groups containing 1-4 carbon atoms), and specifically methyl. A specific example of a substituted thiazole ligand which may be used in accordance with the invention is 5-methylthiazole. The class (ii) dopant preferably is an iridium coordination complex having ligands each of which are more electropositive than a cyano ligand. In a specifically preferred form the remaining non-thiazole or non-substituted-thiazole ligands of the coordination complexes forming class (ii) dopants are halide ligands.

It is specifically contemplated to select class (ii) dopants from among the coordination complexes containing organic ligands disclosed by Olm et al U.S. Pat. No. 5,360,712, Olm et al U.S. Pat. No. 5,457,021 and Kuromoto et al U.S. Pat. No. 5,462,849.

In a preferred form it is contemplated to employ as a class (ii) dopant a hexacoordination complex satisfying the formula:



wherein

$n'$  is zero, -1, -2, -3 or -4; and

$\text{L}_6^1$  represents six bridging ligands which can be independently selected, provided that at least four of the ligands are anionic ligands, each of the ligands is more electropositive than a cyano ligand, and at least one of the ligands comprises a thiazole or substituted thiazole ligand. In a specifically preferred form at least four of the ligands are halide ligands, such as chloride or bromide ligands.

Class (ii) dopant is preferably introduced into the high chloride grains after at least 50 (most preferably 85 and optimally 90) percent of the silver has been precipitated, but before precipitation of the central portion of the grains has been completed. Preferably class (ii) dopant is introduced before 99 (most preferably 97 and optimally 95) percent of the silver has been precipitated. Stated in terms of the fully precipitated grain structure, class (ii) dopant is preferably present in an interior shell region that surrounds at least 50 (most preferably 85 and optimally 90) percent of the silver and, with the more centrally located silver, accounts the entire central portion (99 percent of the silver), most preferably accounts for 97 percent, and optimally accounts for 95 percent of the silver halide forming the high chloride grains. The class (ii) dopant can be distributed throughout the interior shell region delimited above or can be added as one or more bands within the interior shell region.

Class (ii) dopant can be employed in any conventional useful concentration. A preferred concentration range is from  $10^{-9}$  to  $10^{-4}$  mole per silver mole. Iridium is most preferably employed in a concentration range of from  $10^{-8}$  to  $10^{-5}$  mole per silver mole.

Specific illustrations of class (ii) dopants are the following:

- (ii-1)  $[\text{IrCl}_5(\text{thiazole})]^{-2}$
- (ii-2)  $[\text{IrCl}_4(\text{thiazole})_2]^{-1}$
- (ii-3)  $[\text{IrBr}_5(\text{thiazole})]^{-2}$
- (ii-4)  $[\text{IrBr}_4(\text{thiazole})_2]^{-1}$
- (ii-5)  $[\text{IrCl}_5(5\text{-methylthiazole})]^{-2}$
- (ii-6)  $[\text{IrCl}_4(5\text{-methylthiazole})_2]^{-1}$
- (ii-7)  $[\text{IrBr}_5(5\text{-methylthiazole})]^{-2}$
- (ii-8)  $[\text{IrBr}_4(5\text{-methylthiazole})_2]^{-1}$

In one preferred aspect of the invention in a layer using a magenta dye forming coupler, a class (ii) dopant in combination with an  $\text{OsCl}_5(\text{NO})$  dopant has been found to produce a preferred result.

Emulsions demonstrating the advantages of the invention can be realized by modifying the precipitation of conventional high chloride silver halide grains having predominantly (>50%) {100} crystal faces by employing a combination of class (i) and (ii) dopants as described above.

The silver halide grains precipitated contain greater than 50 mole percent chloride, based on silver. Preferably the grains contain at least 70 mole percent chloride and, optimally at least 90 mole percent chloride, based on silver. Iodide can be present in the grains up to its solubility limit, which is in silver iodochloride grains, under typical conditions of precipitation, about 11 mole percent, based on silver. It is preferred for most photographic applications to limit iodide to less than 5 mole percent iodide, most preferably less than 2 mole percent iodide, based on silver.

Silver bromide and silver chloride are miscible in all proportions. Hence, any portion, up to 50 mole percent, of the total halide not accounted for chloride and iodide, can be bromide. For color reflection print (i.e., color paper) uses bromide is typically limited to less than 10 mole percent based on silver and iodide is limited to less than 1 mole percent based on silver.

In a widely used form high chloride grains are precipitated to form cubic grains—that is, grains having {100} major faces and edges of equal length. In practice ripening effects usually round the edges and corners of the grains to some extent. However, except under extreme ripening conditions substantially more than 50 percent of total grain surface area is accounted for by {100} crystal faces.

High chloride tetradecahedral grains are a common variant of cubic grains. These grains contain 6 {100} crystal faces and 8 {111} crystal faces. Tetradecahedral grains are within the contemplation of this invention to the extent that greater than 50 percent of total surface area is accounted for by {100} crystal faces.

Although it is common practice to avoid or minimize the incorporation of iodide into high chloride grains employed in color paper, it is has been recently observed that silver iodochloride grains with {100} crystal faces and, in some instances, one or more {111} faces offer exceptional levels of photographic speed. In the these emulsions iodide is incorporated in overall concentrations of from 0.05 to 3.0 mole percent, based on silver, with the grains having a surface shell of greater than 50 Å that is substantially free of iodide and a interior shell having a maximum iodide concentration that surrounds a core accounting for at least 50 percent of total silver. Such grain structures are illustrated by Chen et al EPO 0 718 679.

In another improved form the high chloride grains can take the form of tabular grains having {100} major faces. Preferred high chloride {100} tabular grain emulsions are those in which the tabular grains account for at least 70 (most preferably at least 90) percent of total grain projected area. Preferred high chloride {100} tabular grain emulsions have average aspect ratios of at least 5 (most preferably at least >8). Tabular grains typically have thicknesses of less than 0.3  $\mu\text{m}$ , preferably less than 0.2  $\mu\text{m}$ , and optimally less than 0.07  $\mu\text{m}$ . High chloride {100} tabular grain emulsions and their preparation are disclosed by Maskasky U.S. Pat.

Nos. 5,264,337 and 5,292,632, House et al U.S. Pat. No. 5,320,938, Brust et al U.S. Pat. No. 5,314,798 and Chang et al U.S. Pat. No. 5,413,904.

Once high chloride grains having predominantly {100} crystal faces have been precipitated with a combination of class (i) and class (ii) dopants described above, chemical and spectral sensitization, followed by the addition of conventional addenda to adapt the emulsion for the imaging application of choice can take any convenient conventional form.

These conventional features are illustrated by Research Disclosure, Item 38957, cited above, particularly:

- III. Emulsion washing;
- IV. Chemical sensitization;
- V. Spectral sensitization and desensitization;
- 15 VI. Antifoggants and stabilizers;
- VII. Absorbing and scattering materials;
- IX. Coating and physical property modifying addenda; and
- X. Dye image formers and modifiers.

Some additional silver halide, typically less than 1 percent, based on total silver, can be introduced to facilitate chemical sensitization. It is also recognized that silver halide can be epitaxially deposited at selected sites on a host grain to increase its sensitivity. For example, high chloride {100} tabular grains with corner epitaxy are illustrated by

25 Maskasky U.S. Pat. No. 5,275,930. For the purpose of providing a clear demarcation, the term "silver halide grain" is herein employed to include the silver necessary to form the grain up to the point that the final {100} crystal faces of the grain are formed. Silver halide later deposited that does not overlie the {100} crystal faces previously formed accounting for at least 50 percent of the grain surface area is excluded in determining total silver forming the silver halide grains. Thus, the silver forming selected site epitaxy is not part of the silver halide grains while silver halide that deposits and provides the final {100} crystal faces of the grains is included in the total silver forming the grains, even when it differs significantly in composition from the previously precipitated silver halide.

Image dye-forming couplers may be included in the element such as couplers that form cyan dyes upon reaction

40 with oxidized color developing agents which are described in such representative patents and publications as: U.S. Pat. Nos. 2,367,531; 2,423,730; 2,474,293; 2,772,162; 2,895,826; 3,002,836; 3,034,892; 3,041,236; 4,883,746 and "Farbkuppler—Eine Literatur Ubersicht," published in

45 Agfa Mitteilungen, Band III, pp. 156–175 (1961). Preferably such couplers are phenols and naphthols that form cyan dyes on reaction with oxidized color developing agent. Also preferable are the cyan couplers described in, for instance, European Patent Application Nos. 491,197; 544,322; 556,700; 556,777; 565,096; 570,006; and 574,948.

50 Typical cyan couplers are represented by the following formulas:



CYAN-1



CYAN-2

-continued



CYAN-3



CYAN-4

wherein  $R_1$ ,  $R_5$  and  $R_8$  each represent a hydrogen or a substituent;  $R_2$  represents a substituent;  $R_3$ ,  $R_4$  and  $R_7$  each represent an electron attractive group having a Hammett's substituent constant  $\sigma_{para}^a$  of 0.2 or more and the sum of the  $\sigma_{para}^a$  values of  $R_3$  and  $R_4$  is 0.65 or more;  $R_6$  represents an electron attractive group having a Hammett's substituent constant  $\sigma_{para}^a$  of 0.35 or more;  $X$  represents a hydrogen or a coupling-off group;  $Z_1$  represents nonmetallic atoms necessary for forming a nitrogen-containing, six-membered, heterocyclic ring which has at least one dissociative group;  $Z_2$  represents  $-\text{C}(R_7)=$  and  $-\text{N}=$ ; and  $Z_3$  and  $Z_4$  each represent  $-\text{C}(R_8)=$  and  $-\text{N}=$ .

For purposes of this invention, an "NB coupler" is a dye-forming coupler which is capable of coupling with the developer 4-amino-3-methyl-N-ethyl-N-(2-methanesulfonamidoethyl) aniline sesquisulfate hydrate to form a dye for which the left bandwidth (LBW) of its absorption spectra upon "spin coating" of a 3% w/v solution of the dye in di-n-butyl sebacate solvent is at least 5 nm. less than the LBW for a 3% w/v solution of the same dye in acetonitrile. The LBW of the spectral curve for a dye is the distance between the left side of the spectral curve and the wavelength of maximum absorption measured at a density of half the maximum.

The "spin coating" sample is prepared by first preparing a solution of the dye in di-n-butyl sebacate solvent (3% w/v). If the dye is insoluble, dissolution is achieved by the addition of some methylene chloride. The solution is filtered and 0.1-0.2 ml is applied to a clear polyethylene terephthalate support (approximately 4 cm x 4 cm) and spun at 4,000 RPM using the Spin Coating equipment, Model No. EC101, available from Headway Research Inc., Garland Tex. The transmission spectra of the so prepared dye samples are then recorded.

Preferred "NB couplers" form a dye which, in n-butyl sebacate, has a LBW of the absorption spectra upon "spin coating" which is at least 15 nm, preferably at least 25 nm, less than that of the same dye in a 3% solution (w/v) in acetonitrile.

In a preferred embodiment the cyan dye-forming "NB coupler" useful in the invention has the formula (IA)



(IA)

wherein

$R'$  and  $R''$  are substituents selected such that the coupler is a "NB coupler", as herein defined; and

$Z$  is a hydrogen atom or a group which can be split off by the reaction of the coupler with an oxidized color developing agent.

The coupler of formula (IA) is a 2,5-diamido phenolic cyan coupler wherein the substituents  $R'$  and  $R''$  are preferably independently selected from unsubstituted or substituted alkyl, aryl, amino, alkoxy and heterocyclic groups.

In a further preferred embodiment, the "NB coupler" has the formula (I):



(I)

wherein

$R'$  and  $R''$  are independently selected from unsubstituted or substituted alkyl, aryl, amino, alkoxy and heterocyclic groups and  $Z$  is as hereinbefore defined;

$R_1$  and  $R_2$  are independently hydrogen or an unsubstituted or substituted alkyl group; and

Typically,  $R'$  is an alkyl, amino or aryl group, suitably a phenyl group.  $R''$  is desirably an alkyl or aryl group or a 5-10 membered heterocyclic ring which contains one or more heteroatoms selected from nitrogen, oxygen and sulfur, which ring group is unsubstituted or substituted.

In the preferred embodiment the coupler of formula (I) is a 2,5-diamido phenol in which the 5-amido moiety is an amide of a carboxylic acid which is substituted in the alpha position by a particular sulfone ( $-\text{SO}_2-$ ) group, such as, for example, described in U.S. Pat. No. 5,686,235. The sulfone moiety is an unsubstituted or substituted alkylsulfone or a heterocyclic sulfone or it is an arylsulfone, which is preferably substituted, in particular in the meta and/or para position.

Couplers having these structures of formulae (I) or (IA) comprise cyan dye-forming "NB couplers" which form image dyes having very sharp-cutting dye hues on the short wavelength side of the absorption curves with absorption maxima ( $\lambda_{max}$ ) which are shifted hypsochromically and are generally in the range of 620-645 nm, which is ideally suited for producing excellent color reproduction and high color saturation in color photographic packaging labels.

Referring to formula (I),  $R_1$  and  $R_2$  are independently hydrogen or an unsubstituted or substituted alkyl group, preferably having from 1 to 24 carbon atoms and in particular 1 to 10 carbon atoms, suitably a methyl, ethyl, n-propyl, isopropyl, butyl or decyl group or an alkyl group substituted with one or more fluoro, chloro or bromo atoms, such as a trifluoromethyl group. Suitably, at least one of  $R_1$  and  $R_2$  is a hydrogen atom and if only one of  $R_1$  and  $R_2$  is a hydrogen atom then the other is preferably an alkyl group having 1 to 4 carbon atoms, more preferably one to three carbon atoms and desirably two carbon atoms.

As used herein and throughout the specification unless where specifically stated otherwise, the term "alkyl" refers to an unsaturated or saturated straight or branched chain alkyl group, including alkenyl, and includes aralkyl and cyclic alkyl groups, including cycloalkenyl, having 3-8 carbon atoms and the term 'aryl' includes specifically fused aryl.

In formula (I),  $R'$  is suitably an unsubstituted or substituted amino, alkyl or aryl group or a 5-10 membered heterocyclic ring which contains one or more heteroatoms

selected from nitrogen, oxygen and sulfur, which ring is unsubstituted or substituted, but is more suitably an unsubstituted or substituted phenyl group.

Examples of suitable substituent groups for this aryl or heterocyclic ring include cyano, chloro, fluoro, bromo, iodo, alkyl- or aryl-carbonyl, alkyl- or aryl-oxycarbonyl, carbonamido, alkyl- or aryl-carbonamido, alkyl- or aryl-sulfonyl, alkyl- or aryl-sulfonyloxy, alkyl- or aryl-oxysulfonyl, alkyl- or aryl-sulfoxide, alkyl- or aryl-sulfamoyl, alkyl- or aryl-sulfonamido, aryl, alkyl, alkoxy, aryloxy, nitro, alkyl- or aryl-ureido and alkyl- or aryl-carbamoyl groups, any of which may be further substituted. Preferred groups are halogen, cyano, alkoxycarbonyl, alkylsulfamoyl, alkyl-sulfonamido, alkylsulfonyl, carbamoyl, alkylcarbamoyl or alkylcarbonamido. Suitably, R" is a 4-chlorophenyl, 3,4-di-chlorophenyl, 3,4-difluorophenyl, 4-cyanophenyl, 3-chloro-4-cyanophenyl, pentafluorophenyl or a 3- or 4-sulfonamidonphenyl group.

In formula (I), when  $R''$  is alkyl it may be unsubstituted or substituted with a substituent such as halogen or alkoxy. When  $R''$  is aryl or a heterocycle, it may be substituted. Desirably it is not substituted in the position alpha to the sulfonyl group.

In formula (I), when R <sup>11</sup> is a phenyl group, it may be substituted in the meta and/or para positions with one to three substituents independently selected from the group consisting of halogen, and unsubstituted or substituted alkyl, alkoxy, aryloxy, acyloxy, acylamino, alkyl- or aryl-sulfonyloxy, alkyl- or aryl-sulfamoyl, alkyl- or aryl-sulfamoylamino, alkyl- or aryl-sulfonamido, alkyl- or arylureido, alkyl- or aryl-oxycarbonyl, alkyl- or aryl-oxy-carbonylamino and alkyl- or aryl-carbamoyl groups.

In particular each substituent may be an alkyl group such as methyl, t-butyl, heptyl, dodecyl, pentadecyl, octadecyl or 1,1,2,2-tetramethylpropyl; an alkoxy group such as methoxy, t-butoxy, octyloxy, dodecyloxy, tetradecyloxy, hexadecyloxy or octadecyloxy; an aryloxy group such as phenoxy, 4-t-butylphenoxy or 4-dodecyl-phenoxy; an alkyl- or aryl-acyloxy group such as acetoxy or dodecanoyloxy; an alkyl- or aryl-acylamino group such as acetamido, hexadecanamido or benzamido; an alkyl- or aryl-sulfonyloxy group such as methyl-sulfonyloxy, dodecylsulfonyloxy or 4-methylphenyl-sulfonyloxy; an alkyl- or aryl-sulfamoyl group such as N-butylsulfamoyl or N-4-t-butylphenylsulfamoyl; an alkyl- or aryl-sulfamoylamino group such as N-butyl-sulfamoylamino or N-4-t-butylphenylsulfamoyl-amino; an alkyl- or aryl-sulfonamido group such as methane-sulfonamido, hexadecanesulfonamido or 4-chlorophenyl-sulfonamido; an alkyl- or aryl-ureido group such as methylureido or phenylureido; an alkoxy- or aryloxy-carbonyl such as methoxycarbonyl or phenoxy carbonyl; an alkoxy- or aryloxy-carbonylamino group such as methoxy-carbonylamino or phenoxy carbonylamino; an alkyl- or aryl-carbamoyl group such as N-butylcarbamoyl or N-methyl-N-dodecylcarbamoyl; or a perfluoroalkyl group such as trifluoromethyl or heptafluoropropyl.

Suitably the above substituent groups have 1 to 30 carbon atoms, more preferably 8 to 20 aliphatic carbon atoms. A desirable substituent is an alkyl group of 12 to 18 aliphatic carbon atoms such as dodecyl, pentadecyl or octadecyl or an alkoxy group with 8 to 18 aliphatic carbon atoms such as dodecyloxy and hexadecyoxy or a halogen such as a meta or para chloro group, carboxy or sulfonamido. Any such groups may contain interrupting heteroatoms such as oxygen to form e.g. polyalkylene oxides.

In formula (I) or (IA) Z is a hydrogen atom or a group which can be split off by the reaction of the coupler with an oxidized color developing agent, known in the photographic art as a 'coupling-off group' and may preferably be 65 hydrogen, chloro, fluoro, substituted aryloxy or mercaptotetrazole, more preferably hydrogen or chloro.

The presence or absence of such groups determines the chemical equivalency of the coupler, i.e., whether it is a 2-equivalent or 4-equivalent coupler, and its particular identity can modify the reactivity of the coupler. Such groups can advantageously affect the layer in which the coupler is coated, or other layers in the photographic recording material, by performing, after release from the coupler, functions such as dye formation, dye hue adjustment, development acceleration or inhibition, bleach acceleration or inhibition, electron transfer facilitation, color correction, and the like.

Representative classes of such coupling-off groups include, for example, halogen, alkoxy, aryloxy, heterocyclyloxy, sulfonyloxy, acyloxy, acyl, heterocyclylsulfonamido, heterocyclylthio, benzothiazolyl, phosphonyloxy, alkylthio, arylthio, and arylazo. These coupling-off groups are described in the art, for example, in U.S. Pat. Nos. 2,455,169, 3,227,551, 3,432,521, 3,467,563, 3,617,291, 3,880,661, 4,052,212, and 4,134,766; and in U.K. Patent Nos. and published applications 1,466,728, 1,531,927, 1,533,039, 2,066,755A, and 2,017,704A, the disclosures of which are incorporated herein by reference. Halogen, alkoxy and aryloxy groups are most suitable.

Examples of specific coupling-off groups are  $-\text{Cl}$ ,  $-\text{F}$ ,  $-\text{Br}$ ,  $-\text{SCN}$ ,  $-\text{OCH}_3$ ,  $-\text{OC}_6\text{H}_5$ ,  $-\text{OCH}_2\text{C}(=\text{O})$ ,  $\text{NHCH}_2\text{CH}_2\text{OH}$ ,  $-\text{OCH}_2\text{C}(\text{O})\text{NHCH}_2\text{CH}_2\text{OCH}_3$ ,  $-\text{OCH}_2\text{C}(\text{O})\text{NHCH}_2\text{CH}_2\text{OC}(=\text{O})\text{OCH}_3$ ,  $-\text{P}(\text{O})(\text{OCH}_2\text{H}_5)_2$ ,  $-\text{SCH}_2\text{CH}_2\text{COOH}$ ,



21

-continued



Typically, the coupling-off group is a chlorine atom, hydrogen atom or p-methoxyphenoxy group. 10

It is essential that the substituent groups be selected so as to adequately ballast the coupler and the resulting dye in the organic solvent in which the coupler is dispersed. The ballasting may be accomplished by providing hydrophobic substituent groups in one or more of the substituent groups. Generally a ballast group is an organic radical of such size and configuration as to confer on the coupler molecule sufficient bulk and aqueous insolubility as to render the coupler substantially nondiffusible from the layer in which it is coated in a photographic element. Thus the combination of substituent are suitably chosen to meet these criteria. To be effective, the ballast will usually contain at least 8 carbon atoms and typically contains 10 to 30 carbon atoms. Suitable ballasting may also be accomplished by providing a plurality of groups which in combination meet these criteria. In the preferred embodiments of the invention  $R_1$  in formula (I) is a small alkyl group or hydrogen. Therefore, in these embodiments the ballast would be primarily located as part of the other groups. Furthermore, even if the coupling-off group  $Z$  contains a ballast it is often necessary to ballast the other substituents as well, since  $Z$  is eliminated from the molecule upon coupling; thus, the ballast is most advantageously provided as part of groups other than  $Z$ .

The following examples further illustrate preferred couplet of the invention. It is not to be construed that the present invention is limited to these examples. 35

3

22

-continued

IC-3



?

2

3

IC 4



4

IC 5



IC 2

5

IC-6



**23**

-continued

IC-7

**24**

-continued

IC-11



IC-8



IC-10



IC-12



IC-13



25

-continued



IC-15

26

-continued



IC-19

IC-16



10



$$\text{CO}_2\text{CH}_3$$



IC-18



65

**27**

-continued

IC-23



IC-24



IC-25



IC-26

**28**

-continued

IC-27



**29**

-continued

IC-31

**30**

-continued

IC-35



IC-32 20



IC-33



IC-36



IC-37



IC-38



IC-34



31

-continued



32

-continued

MAGENTA-2



wherein  $R_a$  and  $R_b$  independently represent H or a substituent;  $R_c$  is a substituent (preferably an aryl group);  $R_d$  is a substituent (preferably an anilino, carbonamido, ureido, carbamoyl, alkoxy, aryloxycarbonyl, alkoxy carbonyl, or 16 N-heterocyclic group); X is hydrogen or a coupling-off group; and  $Z_a$ ,  $Z_b$ , and  $Z_c$  are independently a substituted 17 methine group,  $=N-$ ,  $=C-$ , or  $-NH-$ , provided that one of either the  $Z_a-Z_b$  bond or the  $Z_b-Z_c$  bond is a 18 double bond and the other is a single bond, and when the 19  $Z_b-Z_c$  bond is a carbon-carbon double bond, it may form 20 part of an aromatic ring, and at least one of  $Z_a$ ,  $Z_b$ , and  $Z_c$  represents a methine group connected to the group  $R_b$ .

Specific examples of such couplers are:



MAGENTA-1



Preferred couplers are IC-3, IC-7, IC-35, and IC-36 because of their suitably narrow left bandwidths.

Couplers that form magenta dyes upon reaction with oxidized color developing agent are described in such representative patents and publications as: U.S. Pat. Nos. 2,311, 35 082, 2,343,703, 2,369,489, 2,600,788, 2,908,573, 3,062,653, 3,152,896, 3,519,429, 3,758,309, and "Farbkuppler-eine Literature Ubersicht," published in Agfa Mitteilungen, Band III, pp. 126-156 (1961). Preferably such couplers are pyrazolones, pyrazolotriazoles, or pyrazolobenzimidazoles that form magenta dyes upon reaction with oxidized color developing agents. Especially preferred couplers are 1H-pyrazolo [5,1-c]-1,2,4-triazole 1H-pyrazolo [1,5-b]-1,2, 40 4-triazole. Examples of 1H-pyrazolo [5,1-c]-1,2,4-triazole couplers are described in U.K. Patent Nos. 1,247,493; 1,252, 45 418; 1,398,979, U.S. Pat. Nos. 4,443,536; 4,514,490; 4,540, 654; 4,590,153; 4,665,015; 4,822,730; 4,945,034; 5,017, 465; and 5,023,170. Examples of 1H-pyrazolo [1,5-b]-1,2, 50 4-triazoles can be found in European Patent applications 176,804; 177,765; U.S. Pat. Nos. 4,659,652; 5,066,575; and 5,250,400.

Typical pyrazoloazole and pyrazolone couplers are represented by the following formulas:

33

-continued

## M-5 structures

34

Preferred yellow couplers can be of the following general structures



Couplers that form yellow dyes upon reaction with oxidized color developing agent are described in such representative patents and publications as: U.S. Pat. Nos. 2,298, 443; 2,407,210; 2,875,057; 3,048,194; 3,265,506; 3,447, 928; 3,960,570; 4,022,620; 4,443,536; 4,910,126; and 5,340,703 and "Farbkuppler-eine Literatur Ubersicht," published in Agfa Mitteilungen, Band III, pp. 112-126 (1961). Such couplers are typically open chain ketomethylene compounds. Also preferred are yellow couplers such as described in, for example, European Patent Application Nos. 482,552; 510,535; 524,540; 543,367; and U.S. Pat. No. 5,238,803. For improved color reproduction, couplers which give yellow dyes that cut off sharply on the long wavelength side are particularly preferred (for example, see U.S. Pat. No. 5,360,713).

Typical preferred yellow couplers are represented by the following formulas: 30



wherein  $R_1$ ,  $R_2$ ,  $Q_1$  and  $Q_2$  each represents a substituent;  $X$  is hydrogen or a coupling-off group;  $Y$  represents an aryl group or a heterocyclic group;  $Q_3$  represents an organic residue required to form a nitrogen-containing heterocyclic group together with the  $>N-$ ; and  $Q_4$  represents nonmetallic atoms necessary to form a 3- to 5-membered hydrocarbon ring or a 3- to 5-membered heterocyclic ring which contains at least one hetero atom selected from N, O, S, and P in the ring. Particularly preferred is when  $Q_1$  and  $Q_2$  each represent an alkyl group, an aryl group, or a heterocyclic group, and  $R_2$  represents an aryl or tertiary alkyl group.

35

-continued



Y-6

36

carbamoyl, such as N-methylcarbamoyl, N,N-dibutylcarbamoyl, N-octadecylcarbamoyl, N-[4-(2,4-di-t-pentylphenoxy)butyl]carbamoyl, N-methyl-N-tetradecylcarbamoyl, and N,N-diethylcarbamoyl; acyl, such as acetyl, (2,4-di-t-amylphenoxy)acetyl, phenoxy carbonyl, p-dodecyloxyphenoxy carbonyl, methoxy carbonyl, butoxy carbonyl, tetradecyloxy carbonyl, ethoxy carbonyl, benzyloxy carbonyl, 3-pentadecyloxy carbonyl, and dodecyl oxy carbonyl; sulfonyl, such as methoxysulfonyl, octyloxy sulfonyl, tetradecyloxy sulfonyl, 2-ethylhexyloxy sulfonyl, phenoxy sulfonyl, 2,4-di-t-pentylphenoxy sulfonyl, methylsulfonyl, octylsulfonyl, 2-ethylhexylsulfonyl, dodecylsulfonyl, hexadecylsulfonyl, phenylsulfonyl, 4-nonylphenylsulfonyl, and p-tolylsulfonyl; sulfonyloxy, such as dodecylsulfonyloxy, and hexadecylsulfonyloxy; sulfinyl, such as methylsulfinyl, octylsulfinyl, 2-ethylhexylsulfinyl, dodecylsulfinyl, hexadecylsulfinyl, phenylsulfinyl, 4-nonylphenylsulfinyl, and p-tolylsulfinyl; thio, such as ethylthio, octylthio, benzylthio, tetradecylthio, 2-(2,4-di-t-pentylphenoxy)ethylthio, phenylthio, 2-butoxy-5-t-octylphenylthio, and p-tolylthio; acyloxy, such as acyloxy, benzyloxy, octadecanoxyloxy, p-dodecylamido benzoyloxy, N-phenylcarbamoyloxy, N-ethylcarbamoyloxy, and cyclohexylcarbonyloxy; amino, such as phenylanilino, 2-chloroanilino, diethylamino, dodecylamino; imino, such as 1 (N-phenylimido)ethyl, N-succinimido or 3-benzylhydantoinyl; phosphate, such as dimethylphosphate and ethylbutylphosphate; phosphite, such as diethyl and dihexylphosphite; a heterocyclic group, a heterocyclic oxy group or a heterocyclic thio group, each of which may be substituted and which contain a 3 to 7 membered heterocyclic ring composed of carbon atoms and at least one hetero atom selected from the group consisting of oxygen, nitrogen and sulfur, such as 2-furyl, 2-thienyl, 2-benzimidazolyloxy or 2-benzothiazolyl; quaternary ammonium, such as triethylammonium; and silyloxy, such as trimethylsilyloxy.

If desired, the substituents may themselves be further substituted one or more times with the described substituent groups. The particular substituents used may be selected by those skilled in the art to attain the desired photographic properties for a specific application and can include, for example, hydrophobic groups, solubilizing groups, blocking groups, releasing or releasable groups, etc. Generally, the above groups and substituents thereof may include those having up to 48 carbon atoms, typically 1 to 36 carbon atoms and usually less than 24 carbon atoms, but greater numbers are possible depending on the particular substituents selected.

Representative substituents on ballast groups include alkyl, aryl, alkoxy, aryloxy, alkylthio, hydroxy, halogen, alkoxy carbonyl, arylox carbonyl, carboxy, acyl, acyloxy, amino, anilino, carbonamido, carbamoyl, alkylsulfonyl, arylsulfonyl, sulfonamido, and sulfamoyl groups wherein the substituents typically contain 1 to 42 carbon atoms. Such substituents can also be further substituted.

Silver halide imaging layers substantially free of stabilizers are preferred. Silver halide stabilizers are typically utilized to protect from the growth of fog in storage and to reduce image fading. Stabilizers are however expensive and not generally required for silver halide images attached to packages of the invention since the shelf life of a package tends to be less than one calendar year. Silver halide imaging layers substantially free of stabilizers would be low in cost and have acceptable image quality for images attached to packages.

Stabilizers and scavengers that can be used in these photographic elements, but are not limited to, the following.

Unless otherwise specifically stated, substituent groups which may be substituted on molecules herein include any groups, whether substituted or unsubstituted, which do not destroy properties necessary for photographic utility. When the term "group" is applied to the identification of a substituent containing a substitutable hydrogen, it is intended to encompass not only the substituent's unsubstituted form, but also its form further substituted with any group or groups as herein mentioned. Suitably, the group may be halogen or may be bonded to the remainder of the molecule by an atom of carbon, silicon, oxygen, nitrogen, phosphorous, or sulfur. The substituent may be, for example, halogen, such as chlorine, bromine or fluorine; nitro; hydroxyl; cyano; carboxyl; or groups which may be further substituted, such as alkyl, including straight or branched chain alkyl, such as methyl, trifluoromethyl, ethyl, t-butyl, 3-(2,4-di-t-pentylphenoxy) propyl, and tetradecyl; alkenyl, such as ethylene, 2-butene; alkoxy, such as methoxy, ethoxy, propoxy, butoxy, 2-methoxyethoxy, sec-butoxy, hexyloxy, 2-ethylhexyloxy, tetradecyloxy, 2-(2,4-di-t-pentylphenoxy) ethoxy, and 2-dodecyloxyethoxy; aryl such as phenyl, 4-t-butylphenyl, 2,4,6-trimethylphenyl, naphthyl; aryloxy, such as phenoxy, 2-methylphenoxy, alpha- or beta-naphthoxy, and 4-tolyloxy; carbonamido, such as acetamido, benzamido, butyramido, tetradecanamido, alpha-(2,4-di-t-pentylphenoxy)acetamido, alpha-(2,4-di-t-pentylphenoxy)butyramido, alpha-(3-pentadecylphenoxy)-hexanamido, alpha-(4-hydroxy-3-t-butylphenoxy)-tetradecanamido, 2-oxo-pyrrolidin-1-yl, 2-oxo-5-tetradecylpyrrolin-1-yl, N-methyltetradecanamido, N-succinimido, N-phthalimido, 2,5-dioxo-1-oxazolidinyl, 3-dodecyl-2,5-dioxo-1-imidazolyl, and N-acetyl-N-dodecylamino, ethoxycarbonylamino, phenoxy carbonylamino, benzyloxy carbonylamino, hexadecyloxy carbonylamino, 2,4-di-t-butylphenoxy carbonylamino, phenyl carbonylamino, 2,5-(di-t-pentylphenyl) carbonylamino, p-dodecyl-phenyl carbonylamino, p-tolyl carbonylamino, N-methylureido, N,N-dimethylureido, N-methyl-N-dodecylureido, N-hexadecylureido, N,N-dioctadecylureido, N,N-diethyl-N'-ethylureido, N-phenylureido, N,N-diphenylureido, N-phenyl-N-p-tolylureido, N-(m-hexadecylphenyl)ureido, N,N-(2,5-di-t-pentylphenyl)-N'-ethylureido, and t-butyl carbonamido; sulfonamido, such as methylsulfonamido, benzenesulfonamido, p-tolylsulfonamido, p-dodecylbenzenesulfonamido, N-methyltetradecylsulfonamido, N,N-dipropylsulfamoyl, and hexadecylsulfonamido; sulfamoyl, such as N-methylsulfamoyl, N-ethylsulfamoyl, N,N-dipropylsulfamoyl, N-hexadecylsulfamoyl, N,N-dimethylsulfamoyl; N-[3-(dodecyloxy)propyl]sulfamoyl, N-[4-(2,4-di-t-pentylphenoxy)butyl]sulfamoyl, N-methyl-N-tetradecylsulfamoyl, and N-dodecylsulfamoyl;



ST-1



ST-2



ST-3



ST-4



ST-5



ST-6



ST-7



ST-8



ST-9



ST-10



ST-11



ST-12

**39****40**

-continued

ST-13

ST-14



ST-15



ST-16



ST-17



ST-18



ST-19



ST-20

 $n = 75-8,000$ 

ST-21



ST-22



n:m 1:1 mw = 75-100,000

-continued  
ST-23

ST-24

20

Examples of solvents which may be used in the invention include the following:

|                                                 |      |
|-------------------------------------------------|------|
| Tritolyl phosphate                              | S-1  |
| Dibutyl phthalate                               | S-2  |
| Diundecyl phthalate                             | S-3  |
| N,N-Diethyldodecanamide                         | S-4  |
| N,N-Dibutyldodecanamide                         | S-5  |
| Tris(2-ethylhexyl)phosphate                     | S-6  |
| Acetyl tributyl citrate                         | S-7  |
| 2,4-Di-tert-pentylphenol                        | S-8  |
| 2-(2-Butoxyethoxy)ethyl acetate                 | S-9  |
| 1,4-Cyclohexyldimethylene bis(2-ethylhexanoate) | S-10 |

25



UV-3



UV-4

45  
UV-1

UV-5

50  
UV-2

UV-6



65

The dispersions used in photographic elements may also include ultraviolet (UV) stabilizers and so called liquid UV 40 stabilizers such as described in U.S. Pat. Nos. 4,992,358; 4,975,360; and 4,587,346. Examples of UV stabilizers are shown below.

43

-continued



44

-continued

UV-7 SF-10

5 SF-11

UV-8 SF-12

10

15 SF-12



The aqueous phase may include surfactants. Surfactant may be cationic, anionic, zwitterionic or non-ionic. Useful surfactants include, but are not limited to, the following.



$\text{CF}_3\text{-}(\text{CF}_2)_7\text{-SO}_3\text{Na}$

$\text{CH}_3\text{-}(\text{CH}_2)_n\text{-SO}_3\text{Na}$ ,  $n = 12-14$

Further, it is contemplated to stabilize photographic dispersions prone to particle growth through the use of hydrophobic, photographically inert compounds such as disclosed by Zengerle et al in U.S. Ser. No. 07/978,104.

In a preferred embodiment the invention employs recording elements which are constructed to contain at least three silver halide emulsion layer units. A suitable full color, multilayer format for a recording element used in the invention is represented by Structure I.

SF-4



$\text{CH}_3\text{-}(\text{CH}_2)_11\text{-OSO}_3\text{Na}$

35 Red-sensitized  
cyan dye image-forming silver halide emulsion unit  
Interlayer

40 Green-sensitized  
magenta dye image-forming silver halide emulsion unit  
Interlayer

45 Blue-sensitized  
yellow dye image-forming silver halide emulsion unit  
//// Duplitzed Imaging Base ////

50 Red-sensitized  
cyan dye image-forming silver halide emulsion unit  
Interlayer

55 Green-sensitized  
magenta dye image-forming silver halide emulsion unit  
Interlayer

60 Blue-sensitized  
yellow dye image forming silver halide emulsion unit

Structure I

wherein the topside red-sensitized, cyan dye image-forming silver halide emulsion unit is situated furthest from the polymer base; next in order is the green-sensitized, magenta dye image-forming unit, followed by the lowermost blue-sensitized, yellow dye image-forming unit. The image-forming units are separated from each other by hydrophilic colloid interlayers containing an oxidized developing agent scavenger to prevent color contamination. Silver halide emulsions satisfying the grain and gelatino-peptizer requirements described above can be present in any one or combination of the emulsion layer units. Additional useful multicolor, multilayer formats for an element of the invention include structures as described in U.S. Pat. No. 5,783,373. Each of such structures in accordance with the invention preferably would contain at least three silver halide emulsions comprised of high chloride grains having at least



$n = \text{ca. } 6, m = \text{ca. } 2$



$n = \text{ca. } 6, m = \text{ca. } 2$

50 percent of their surface area bounded by {100} crystal faces and containing dopants from classes (i) and (ii), as described above. Preferably each of the emulsion layer units contains emulsion satisfying these criteria.

Conventional features that can be incorporated into multilayer (and particularly multicolor) recording elements contemplated for use in the method of the invention are illustrated by *Research Disclosure*, Item 38957, cited above:

- XI. Layers and layer arrangements
- XII. Features applicable only to color negative
- XIII. Features applicable only to color positive
  - B. Color reversal
  - C. Color positives derived from color negatives
- XIV. Scan facilitating features.

The recording elements comprising the radiation sensitive high chloride emulsion layers according to this invention can be conventionally optically printed, or in accordance with a particular embodiment of the invention can be image-wise exposed in a pixel-by-pixel mode using suitable high energy radiation sources typically employed in electronic printing methods. Suitable actinic forms of energy encompass the ultraviolet, visible and infrared regions of the electromagnetic spectrum as well as electron-beam radiation and is conveniently supplied by beams from one or more light emitting diodes or lasers, including gaseous or solid state lasers. Exposures can be monochromatic, orthochromatic or panchromatic. For example, when the recording element is a multilayer multicolor element, exposure can be provided by laser or light emitting diode beams of appropriate spectral radiation, for example, infrared, red, green or blue wavelengths, to which such element is sensitive. Multicolor elements can be employed which produce cyan, magenta and yellow dyes as a function of exposure in separate portions of the electromagnetic spectrum, including at least two portions of the infrared region, as disclosed in the previously mentioned U.S. Pat. No. 4,619,892. Suitable exposures include those up to 2000 nm, preferably up to 1500 nm. Suitable light emitting diodes and commercially available laser sources are known and commercially available. Imagewise exposures at ambient, elevated or reduced temperatures and/or pressures can be employed within the useful response range of the recording element determined by conventional sensitometric techniques, as illustrated by T. H. James, *The Theory of the Photographic Process*, 4th Ed., Macmillan, 1977, Chapters 4, 6, 17, 18 and 23.

It has been observed that anionic  $[MX_xY_yL_z]$  hexacoordination complexes, where M is a group 8 or 9 metal (preferably iron, ruthenium or iridium), X is halide or pseudohalide (preferably Cl, Br or CN) x is 3 to 5, Y is  $H_2O$ , y is 0 or 1, L is a C—C, H—C or C—N—H organic ligand, and Z is 1 or 2, are surprisingly effective in reducing high intensity reciprocity failure (HIRF), low intensity reciprocity failure (LIRF) and thermal sensitivity variance and in improving latent image keeping (LIK). As herein employed HIRF is a measure of the variance of photographic properties for equal exposures, but with exposure times ranging from  $10^{-1}$  to  $10^{-6}$  second. LIRF is a measure of the variance of photographic properties for equal exposures, but with exposure times ranging from  $10^{-1}$  to 100 seconds. Although these advantages can be generally compatible with face centered cubic lattice grain structures, the most striking improvements have been observed in high (>50 mole %, preferably  $\geq 90$  mole %) chloride emulsions. Preferred C—C, H—C or C—N—H organic ligands are aromatic heterocycles of the type described in U.S. Pat. No. 5,462,849. The most effective C—C, H—C or C—N—H organic ligands are azoles and azines, either unsubstituted or contain-

ing alkyl, alkoxy or halide substituents, where the alkyl moieties contain from 1 to 8 carbon atoms. Particularly preferred azoles and azines include thiazoles, thiazolines and pyrazines.

The quantity or level of high energy actinic radiation provided to the recording medium by the exposure source is generally at least  $10^{-4}$  ergs/cm<sup>2</sup>, typically in the range of about  $10^{-4}$  ergs/cm<sup>2</sup> to  $10^{-3}$  ergs/cm<sup>2</sup> and often from  $10^{-3}$  ergs/cm<sup>2</sup> to  $10^{-2}$  ergs/cm<sup>2</sup>. Exposure of the recording element in a pixel-by-pixel mode as known in the prior art persists for only a very short duration or time. Typical maximum exposure times are up to  $100\mu$  seconds, often up to  $10\mu$  seconds, and frequently up to only  $0.5\mu$  seconds. Single or multiple exposures of each pixel are contemplated. The pixel density is subject to wide variation, as is obvious to those skilled in the art. The higher the pixel density, the sharper the images can be, but at the expense of equipment complexity. In general, pixel densities used in conventional electronic printing methods of the type described herein do not exceed  $10^7$  pixels/cm<sup>2</sup> and are typically in the range of about  $10^4$  to  $10^6$  pixels/cm<sup>2</sup>. An assessment of the technology of high-quality, continuous-tone, color electronic printing using silver halide photographic paper which discusses various features and components of the system, including exposure source, exposure time, exposure level and pixel density and other recording element characteristics is provided in Firth et al., *A Continuous-Tone Laser Color Printer*, Journal of Imaging Technology, Vol. 14, No. 3, June 1988, which is hereby incorporated herein by reference. As previously indicated herein, a description of some of the details of conventional electronic printing methods comprising scanning a recording element with high energy beams such as light emitting diodes or laser beams, are set forth in Hioki U.S. Pat. No. 5,126,235, European Patent Applications 479 167 A1 and 502 508 A1.

Once imagewise exposed, the recording elements can be processed in any convenient conventional manner to obtain a viewable image. Such processing is illustrated by *Research Disclosure*, Item 38957, cited above:

- XVIII. Chemical development systems
- XIX. Development
- XX. Desilvering, washing, rinsing and stabilizing

In addition, a useful developer for the inventive material is a homogeneous, single part developing agent. The homogeneous, single-part color developing concentrate is prepared using a critical sequence of steps:

In the first step, an aqueous solution of a suitable color developing agent is prepared. This color developing agent is generally in the form of a sulfate salt. Other components of the solution can include an antioxidant for the color developing agent, a suitable number of alkali metal ions (in an at least stoichiometric proportion to the sulfate ions) provided by an alkali metal base, and a photographically inactive water-miscible or water-soluble hydroxy-containing organic solvent. This solvent is present in the final concentrate at a concentration such that the weight ratio of water to the organic solvent is from about 15:85 to about 50:50.

In this environment, especially at high alkalinity, alkali metal ions and sulfate ions form a sulfate salt that is precipitated in the presence of the hydroxy-containing organic solvent. The precipitated sulfate salt can then be readily removed using any suitable liquid/solid phase separation technique (including filtration, centrifugation or decantation). If the antioxidant is a liquid organic compound, two phases may be formed and the precipitate may be removed by discarding the aqueous phase.

The color developing concentrates of this invention include one or more color developing agents that are well

known in the art that, in oxidized form, will react with dye forming color couplers in the processed materials. Such color developing agents include, but are not limited to, aminophenols, p-phenylenediamines (especially N,N-dialkyl-p-phenylenediamines) and others which are well known in the art, such as EP 0 434 097A1 (published Jun. 26, 1991) and EP 0 530 921A1 (published Mar. 10, 1993). It may be useful for the color developing agents to have one or more water-solubilizing groups as are known in the art. Further details of such materials are provided in *Research Disclosure*, publication 38957, pages 592-639 (September 1996). *Research Disclosure* is a publication of Kenneth Mason Publications Ltd., Dudley House, 12 North Street, Emsworth, Hampshire PO10 7DQ England (also available from Emsworth Design Inc., 121 West 19th Street, New York, N.Y. 10011). This reference will be referred to hereinafter as "Research Disclosure".

Preferred color developing agents include, but are not limited to, N,N-diethyl p-phenylenediamine sulfate (KODAK Color Developing Agent CD-2), 4-amino-3-methyl-N-(2-methane sulfonamidoethyl)aniline sulfate, 4-(N-ethyl-N-β-hydroxyethylamino)-2-methylaniline sulfate (KODAK Color Developing Agent CD-4), p-hydroxyethylaminoaniline sulfate, 4-(N-ethyl-N-2-methanesulfonylaminoethyl)-2-methylphenylenediamine sesquisulfate (KODAK Color Developing Agent CD-3), 4-(N-ethyl-N-2-methanesulfonylaminoethyl)-2-methylphenylenediamine sesquisulfate, and others readily apparent to one skilled in the art.

In order to protect the color developing agents from oxidation, one or more antioxidants are generally included in the color developing compositions. Either inorganic or organic antioxidants can be used. Many classes of useful antioxidants are known, including but not limited to, sulfites (such as sodium sulfite, potassium sulfite, sodium bisulfite and potassium metabisulfite), hydroxylamine (and derivatives thereof), hydrazines, hydrazides, amino acids, ascorbic acid (and derivatives thereof), hydroxamic acids, aminoketones, mono- and polysaccharides, mono- and polyamines, quaternary ammonium salts, nitroxy radicals, alcohols, and oximes. Also useful as antioxidants are 1,4-cyclohexadienes. Mixtures of compounds from the same or different classes of antioxidants can also be used if desired.

Especially useful antioxidants are hydroxylamine derivatives as described for example, in U.S. Pat. Nos. 4,892,804, 4,876,174, 5,354,646, and 5,660,974, all noted above, and U.S. Pat. No. 5,646,327 (Burns et al). Many of these antioxidants are mono- and dialkylhydroxylamines having one or more substituents on one or both alkyl groups. Particularly useful alkyl substituents include sulfo, carboxy, amino, sulfonamido, carbonamido, hydroxy and other solubilizing substituents.

More preferably, the noted hydroxylamine derivatives can be mono- or dialkylhydroxylamines having one or more hydroxy substituents on the one or more alkyl groups. Representative compounds of this type are described for example in U.S. Pat. No. 5,709,982 (Marrese et al), incorporated herein by reference, as having the structure I:



wherein R is hydrogen, a substituted or unsubstituted alkyl group of 1 to 10 carbon atoms, a substituted or unsubstituted hydroxyalkyl group of 1 to 10 carbon atoms, a substituted or unsubstituted cycloalkyl group of 5 to 10 carbon atoms, or

a substituted or unsubstituted aryl group having 6 to 10 carbon atoms in the aromatic nucleus.

X<sub>1</sub> is —CR<sub>2</sub>(OH)CHR<sub>1</sub>— and X<sub>2</sub> is —CHR<sub>1</sub>CR<sub>2</sub>(OH)— wherein R<sub>1</sub> and R<sub>2</sub> are independently hydrogen, hydroxy, a substituted or unsubstituted alkyl group or 1 or 2 carbon atoms, a substituted or unsubstituted hydroxyalkyl group of 1 or 2 carbon atoms, or R<sub>1</sub> and R<sub>2</sub> together represent the carbon atoms necessary to complete a substituted or unsubstituted 5- to 8-membered saturated or unsaturated carbocyclic ring structure.

Y is a substituted or unsubstituted alkylene group having at least 4 carbon atoms, and has an even number of carbon atoms, or Y is a substituted or unsubstituted divalent aliphatic group having an even total number of carbon and oxygen atoms in the chain, provided that the aliphatic group has a least 4 atoms in the chain.

Also in Structure I, m, n and p are independently 0 or 1. Preferably, each of m and n is 1, and p is 0.

Specific di-substituted hydroxylamine antioxidants include, but are not limited to: N,N-bis(2,3-dihydroxypropyl)hydroxylamine, N,N-bis(2-methyl-2,3-dihydroxypropyl)hydroxylamine and N,N-bis(1-hydroxymethyl-2-hydroxy-3-phenylpropyl)hydroxylamine. The first compound is preferred.

The colorants can be incorporated into the imaging element by direct addition of the colorant to a coating melt by mixing the colorant with an aqueous medium containing gelatin (or other hydrophilic colloid) at a temperature of 40° C. or higher. The colorant can also be mixed with an aqueous solution of a water-soluble or water-dispersible surfactant or polymer, and passing the premix through a mill until the desired particle size is obtained. The mill can be any high energy device such as a colloid mill, high pressure homogenizer, or the like.

The preferred color of the pigment is blue as a blue pigment incorporated into a gelatin layer offsets the native yellowness of the gelatin yielding a neutral background for the image layers.

Suitable pigments used in this invention can be any inorganic or organic, colored materials which are practically insoluble in the medium in which they are incorporated. The preferred pigments are organic, and are those described in *Industrial Organic Pigments: Production, Properties, Applications* by W. Herbst and K. Hunger, 1993, Wiley Publishers. These include: Azo Pigments such as monoazo yellow and orange, diazo, naphthol, naphthol reds, azo lakes, benzimidazolone, disazo condensation, metal complex, isoindolinone and isoindoline, Polycyclic Pigments such as phthalocyanine, quinacridone, perylene, perinone, diketopyrrolo pyrrole and thioindigo, and Anthrquinone Pigments such as anthrapyrimidine, flavanthrone, pyranthrone, anthanthrone, dioxazine, triarylcarbodium and quinophthalone.

The most preferred pigments are the anthraquinones such as Pigment Blue 60, phthalocyanines such as Pigment Blue 15, 15:1, 15:3, 15:4 and 15:6, and quinacridones such as Pigment Red 122, as listed in *NPIRI Raw Materials Data Handbook*, Vol. 4, Pigments, 1983, National Printing Research Institute. These pigments have a dye hue sufficient to overcome the native yellowness of the gelatin imaging layer and are easily dispersed in a aqueous solution.

An aqueous dispersion of the pigments is preferred because the preferred pigments are insoluble in most, if not all, organic solvents, and therefore a high quality dispersion is not likely in a solvent system. In fact, the only solvent that will dissolve preferred pigments PR-122 and PB-15 is concentrated sulfuric acid, which is not an organic solvent.

Preferred pigments of the invention are by nature, insoluble, crystalline solids, which is the most thermodynamically stable form that they can assume. In an oil and water dispersion, they would be in the form of an amorphous solid, which is thermodynamically unstable. Therefore, one would have to worry about the pigment eventually converting to the crystalline form with age. We might as well start with a crystalline solid and not worry about preventing the phase transition. Another reason to avoid solvent pigment dispersions is that the high boiling solvent is not removed with evaporation, and it could cause unwanted interactions in the coating melt such as ripening of DOH dispersion particles, or equilibration with other layers, if it was used in the coating. The use of solid particle dispersion avoids organic solvents altogether.

In the preferred embodiment, the colorant is dispersed in the binder in the form of a solid particle dispersion. Such dispersions are formed by first mixing the colorant with an aqueous solution containing a water-soluble or water-dispersible surfactant or polymer to form a coarse aqueous premix, and adding the premix to a mill. The amount of water-soluble or water-dispersible surfactant or polymer can vary over a wide range, but is generally in the range of 0.01% to 100% by weight of polymer, preferably about 0.3% to about 60%, and more preferably 0.5% to 50%, the percentages being by weight of polymer, based on the weight of the colorant useful in imaging.

The mill can be for example, a ball mill, media mill, attritor mill, vibratory mill or the like. The mill is charged with the appropriate milling media such as, for example, beads of silica, silicon nitride, sand, zirconium oxide, yttria-stabilized zirconium oxide, alumina, titanium, glass, polystyrene, etc. The bead sizes typically range from 0.25 to 3.0 mm in diameter, but smaller media can be used if desired. The premix is milled until the desired particle size range is reached.

The solid colorant particles are subjected to repeated collisions with the milling media, resulting in crystal fracture, deagglomeration, and consequent particle size reduction. The solid particle dispersions of the colorant should have a final average particle size of less than 1 micrometers, preferably less than 0.1 micrometers, and most preferably between 0.01 and 0.1 micrometers. Most preferably, the solid colorant particles are of sub-micrometer average size. Solid particle size between 0.01 and 0.1 provides the best pigment utilization and had a reduction in unwanted light absorption compared to pigments with a particle size greater than 1.2 micrometers.

Surfactants, polymers, and other additional conventional addenda may also be used in the dispersing process described herein in accordance with prior art solid particle dispersing procedures. Such surfactants, polymers and other addenda are disclosed in U.S. Pat. Nos. 5,468,598, 5,300, 394, 5,278,037, 4,006,025, 4,924,916, 4,294,917, 4,940,654, 4,950,586, 4,927,744, 5,279,931, 5,158,863, 5,135,844, 5,091,296, 5,089,380, 5,103,640, 4,990,431, 4,970,139, 5,256,527, 5,089,380, 5,103,640, 4,990,431, 4,970,139, 5,256,527, 5,015,564, 5,008,179, 4,957,857, and 2,870,012, British Patent specifications Nos. 1,570,362 and 1,131,179 referenced above, the disclosures of which are hereby incorporated by reference, in the dispersing process of the colorants.

Additional surfactants or other water soluble polymers may be added after formation of the colorant dispersion, before or after subsequent addition of the colorant dispersion to an aqueous coating medium for coating onto a polymer base. The aqueous medium preferably contains other com-

pounds such as stabilizers and dispersants, for example, additional anionic, nonionic, zwitterionic, or cationic surfactants, and water soluble binders such as gelatin as is well known in the imaging art. The aqueous coating medium may further contain other dispersions or emulsions of compounds useful in imaging.

The following examples illustrate the practice of this invention. They are not intended to be exhaustive of all possible variations of the invention. Parts and percentages are by weight unless otherwise indicated.

## EXAMPLES

### Example 1

15 In this example a reflective duplitzited silver halide image was made by coating a light sensitive silver halide emulsion on both sides of a white reflecting base that contained an integral polyethylene layer used to promote silver halide emulsion. The same biaxially oriented polymer sheet was 20 laminated to both the top and bottom sides of a cellulose paper. A gas voided polymer layer in combination with layers containing  $TiO_2$  were utilized to provide the imaging base opacity to reduce unwanted exposure of the opposite side imaging layers during the exposure step. This example 25 will demonstrate a superior duplitzited silver halide image compared to prior art methods of post process adhesion of two photographs together. Further, this example will show that by post process lamination of the processed image layers, that the images are protected from handling and 30 viewing damage common to album pages.

The following is a description of photographic support material (invention) and was prepared by extrusion laminating the following top and bottom biaxially oriented polymer sheets to the cellulose paper described below:

#### Top and Bottom Biaxially Oriented Polymer Sheet

35 A composite sheet consisting of 5 layers identified as L1, L2, L3, L4, and L5. L1 is the thin colored layer on the outside of the package to which the photosensitive silver halide layer was attached. L2 is the layer to which optical brightener and  $TiO_2$  was added. The optical brightener used was Hostalux KS manufactured by Ciba-Geigy. The rutile  $TiO_2$  used was DuPont R104 (a 0.22  $\mu m$  particle size  $TiO_2$ ). Table 1 below lists the characteristics of the layers of the top 40 biaxially oriented sheet used in this example.

TABLE 1

| Layer | Material                            | Thickness, $\mu m$ |
|-------|-------------------------------------|--------------------|
| L1    | LD Polyethylene + color concentrate | 0.75               |
| L2    | Polypropylene + 24% $TiO_2$         | 4.6                |
| L3    | Voided Polypropylene                | 25.1               |
| L4    | Polypropylene + 24% $TiO_2$         | 4.6                |
| L5    | Polypropylene                       | 0.76               |

50 Paper base was produced for photographic base of the invention using a standard fourdrinier paper machine and a blend of mostly bleached hardwood Kraft fibers. The fiber ratio consisted primarily of bleached poplar (38%) and maple/beech (37%) with lesser amounts of birch (18%) and softwood (7%). Fiber length was reduced from 0.73 mm length weighted average as measured by a Kajaani FS-200 to 0.55 mm length using high levels of conical refining and low levels of disc refining. Fiber Lengths from the slurry were measured using a FS-200 Fiber Length Analyzer (Kajaani Automation Inc.). Energy applied to the fibers indicated by the total Specific Net Refining Power (SNRP) was 115 KW hr/metric ton. Two conical refiners were used 55 60 65

in series to provide the total conical refiners SNRP value. This value was obtained by adding the SNRPs of each conical refiner. Two disc refiners were similarly used in series to provide a total Disk SNRP. Neutral sizing chemical addenda, utilized on a dry weight basis, included alkyl ketene dimer at 0.20% addition, cationic starch (1.0%), polyaminoamide epichlorhydrin (0.50%), polyacrylamide resin (0.18%), diaminostilbene optical brightener (0.20%), and sodium bicarbonate. Surface sizing using hydroxyethylated starch and sodium chloride was also employed but is not critical to the invention. In the 3<sup>rd</sup> Dryer section, ratio drying was utilized to provide a moisture bias from the face side to the wire side of the sheet. The face side (emulsion side) of the sheet was then remoisturized with conditioned steam immediately prior calendering. Sheet temperatures were raised to between 76° C. and 93° C. just prior to and during calendering. The paper was then calendered to an apparent density of 1.06 moisture levels after the calender was 7.0% to 9.0% by weight. Paper base A was produced at a basis weight of 127 g/m<sup>2</sup> and thickness of 0.1194 mm.

The top sheet and bottom sheet used in this example was coextruded and biaxially oriented. The top and bottom sheet was melt extrusion laminated to the above cellulose paper base using a metallocene catalyzed ethylene plastomer (Exxon SLP 9088 manufactured by Exxon Chemical Corp.). The metallocene catalyzed ethylene plastomer had a density of 0.900 g/cc and a melt index of 14.0.

The L3 layer for the top and bottom biaxially oriented sheet is microvoided and further described in Table 2 where the refractive index and geometrical thickness is shown for measurements made along a single slice through the L3 layer; they do not imply continuous layers; a slice along another location would yield different but approximately the same thickness. The areas with a refractive index of 1.0 are voids that are filled with air and the remaining layers are polypropylene polymer.

TABLE 2

| Sublayer of L3 | Refractive Index | Thickness, $\mu\text{m}$ |
|----------------|------------------|--------------------------|
| 1              | 1.49             | 2.54                     |
| 2              | 1                | 1.527                    |
| 3              | 1.49             | 2.79                     |
| 4              | 1                | 1.016                    |
| 5              | 1.49             | 1.778                    |
| 6              | 1                | 1.016                    |
| 7              | 1.49             | 2.286                    |
| 8              | 1                | 1.016                    |
| 9              | 1.49             | 2.032                    |
| 10             | 1                | 0.762                    |
| 11             | 1.49             | 2.032                    |
| 12             | 1                | 1.016                    |
| 13             | 1.49             | 1.778                    |
| 14             | 1                | 1.016                    |
| 15             | 1.49             | 2.286                    |

Silver chloride emulsions were chemically and spectrally sensitized as described below. A biocide comprising a mixture of N-methyl-isothiazolone and N-methyl-5-chloroisothiazolone was added after sensitization.

#### Blue Sensitive Emulsion (Blue EM-1)

A high chloride silver halide emulsion is precipitated by adding approximately equimolar silver nitrate and sodium chloride solutions into a well stirred reactor containing glutaryldiaminophenylsulfide, gelatin peptizer and thioether ripener. Cesium pentachloronitrosylsulfate(II) dopant is added during the silver halide grain formation for most of the precipitation, followed by the addition of potassium hexacyanoruthenate(II), potassium (5-methylthiazole)-pentachloroiodate, a small amount of KI solution, and

shelling without any dopant. The resultant emulsion contains cubic shaped grains having edge length of 0.6  $\mu\text{m}$ . The emulsion is optimally sensitized by the addition of a colloidal suspension of aurous sulfide and heat ramped to 60° C. during which time blue sensitizing dye BSD-4, potassium hexachloroiodate, Lippmann bromide and 1-(3-acetamidophenyl)-5-mercaptopotetrazole were added.

#### Green Sensitive Emulsion (Green EM-1)

A high chloride silver halide emulsion is precipitated by adding approximately equimolar silver nitrate and sodium chloride solutions into a well stirred reactor containing, gelatin peptizer and thioether ripener. Cesium pentachloronitrosylsulfate(II) dopant is added during the silver halide grain formation for most of the precipitation, followed by the addition of potassium (5-methylthiazole)-pentachloroiodate. The resultant emulsion contains cubic shaped grains of 0.3  $\mu\text{m}$  in edgewidth size. The emulsion is optimally sensitized by the addition of glutaryldiaminophenylsulfide, a colloidal suspension of aurous sulfide and heat ramped to 55° C. during which time potassium hexachloroiodate doped Lippmann bromide, a liquid crystalline suspension of green sensitizing dye GSD-1, and 1-(3-acetamidophenyl)-5-mercaptopotetrazole were added.

#### Red Sensitive Emulsion (Red EM-1)

A high chloride silver halide emulsion is precipitated by adding approximately equimolar silver nitrate and sodium chloride solutions into a well stirred reactor containing gelatin peptizer and thioether ripener. During the silver halide grain formation, potassium hexacyanoruthenate(II) and potassium (5-methylthiazole)-pentachloroiodate are added. The resultant emulsion contains cubic shaped grains of 0.4  $\mu\text{m}$  in edgewidth size. The emulsion is optimally sensitized by the addition of glutaryldiaminophenylsulfide, sodium thiosulfate, tripotassium bis{2-[3-(2-sulfobenzamido)phenyl]-mercaptopotetrazole} gold(I) and heat ramped to 64° C. during which time 1-(3-acetamidophenyl)-5-mercaptopotetrazole, potassium hexachloroiodate, and potassium bromide are added. The emulsion is then cooled to 40° C., pH adjusted to 6.0 and red sensitizing dye RSD-1 is added.

The following light sensitive silver halide imaging layers were utilized to prepare photographic duplitzed image. The following imaging layers were coated on both sides of the support utilizing curtain coating:

| Layer   | Item                                                                      | Laydown (g/m <sup>2</sup> ) |
|---------|---------------------------------------------------------------------------|-----------------------------|
| Layer 1 | Blue Sensitive Layer                                                      |                             |
|         | Gelatin                                                                   | 1.3127                      |
|         | Blue sensitive silver (Blue EM-1)                                         | 0.2399                      |
|         | Y-4                                                                       | 0.4143                      |
|         | ST-23                                                                     | 0.4842                      |
|         | Tributyl Citrate                                                          | 0.2179                      |
|         | ST-24                                                                     | 0.1211                      |
|         | ST-16                                                                     | 0.0095                      |
|         | Sodium Phenylmercaptopotetrazole                                          | 0.0001                      |
|         | Piperidino hexose reductone                                               | 0.0024                      |
|         | 5-chloro-2-methyl-4-isothiazolin-3-one/2-methyl-4-isothiazolin-3-one(3/1) | 0.0002                      |
|         | SF-1                                                                      | 0.0366                      |
|         | Potassium chloride                                                        | 0.0204                      |
|         | Dye-1                                                                     | 0.0148                      |
| Layer 2 | Interlayer                                                                |                             |
|         | Gelatin                                                                   | 0.7532                      |
|         | ST-4                                                                      | 0.1076                      |
|         | S-3                                                                       | 0.1969                      |

-continued

| Layer   | Item                                                                      | Laydown (g/m <sup>2</sup> ) |
|---------|---------------------------------------------------------------------------|-----------------------------|
|         | 5-chloro-2-methyl-4-isothiazolin-3-one/2-methyl-4-isothiazolin-3-one(3/1) | 0.0001                      |
|         | Catechol disulfonate                                                      | 0.0323                      |
|         | SF-1                                                                      | 0.0081                      |
| Layer 3 | Green Sensitive Layer                                                     |                             |
|         | Gelatin                                                                   | 1.1944                      |
|         | 1)                                                                        | 0.1011                      |
|         | M-4                                                                       | 0.2077                      |
|         | Oleyl Alcohol                                                             | 0.2174                      |
|         | S-3                                                                       | 0.1119                      |
|         | ST-21                                                                     | 0.0398                      |
|         | ST-22                                                                     | 0.2841                      |
|         | Dye-2                                                                     | 0.0073                      |
|         | 5-chloro-2-methyl-4-isothiazolin-3-one/2-methyl-4-isothiazolin-3-one(3/1) | 0.0001                      |
|         | SF-1                                                                      | 0.0236                      |
|         | Potassium chloride                                                        | 0.0204                      |
|         | Sodium Phenylmercaptotetrazole                                            | 0.0007                      |
| Layer 4 | M/C Interlayer                                                            |                             |
|         | Gelatin                                                                   | 0.7532                      |
|         | ST-4                                                                      | 0.1076                      |
|         | S-3                                                                       | 0.1969                      |
|         | Acrylamide/t-Butylacrylamide sulfonate copolymer                          | 0.0541                      |
|         | Bis-vinylsulfonylmethane                                                  | 0.1390                      |
|         | 3,5-Dinitrobenzoic acid                                                   | 0.0001                      |
|         | Citric acid                                                               | 0.0007                      |
|         | Catechol disulfonate                                                      | 0.0323                      |
|         | 5-chloro-2-methyl-4-isothiazolin-3-one/2-methyl-4-isothiazolin-3-one(3/1) | 0.0001                      |
| Layer 5 | Red Sensitive Layer                                                       |                             |
|         | Gelatin                                                                   | 1.3558                      |
|         | Red Sensitive silver (Red EM-1)                                           | 0.1883                      |
|         | IC-35                                                                     | 0.2324                      |
|         | IC-36                                                                     | 0.0258                      |
|         | UV-2                                                                      | 0.3551                      |
|         | Dibutyl sebacate                                                          | 0.4358                      |
|         | S-6                                                                       | 0.1453                      |
|         | Dye-3                                                                     | 0.0229                      |
|         | Potassium p-toluenethiosulfonate                                          | 0.0026                      |
|         | 5-chloro-2-methyl-4-isothiazolin-3-one/2-methyl-4-isothiazolin-3-one(3/1) | 0.0001                      |
|         | Sodium Phenylmercaptotetrazole                                            | 0.0005                      |
|         | SF-1                                                                      | 0.0524                      |
| Layer 6 | UV Overcoat                                                               |                             |
|         | Gelatin                                                                   | 0.8231                      |
|         | UV-1                                                                      | 0.0355                      |
|         | UV-2                                                                      | 0.2034                      |
|         | ST-4                                                                      | 0.0655                      |
|         | SF-1                                                                      | 0.0125                      |
|         | S-6                                                                       | 0.0797                      |
|         | 5-chloro-2-methyl-4-isothiazolin-3-one/2-methyl-4-isothiazolin-3-one(3/1) | 0.0001                      |
| Layer 7 | SOC                                                                       |                             |
|         | Gelatin                                                                   | 0.6456                      |
|         | Ludox AM™ (colloidal silica)                                              | 0.1614                      |
|         | Polydimethylsiloxane (DC200™)                                             | 0.0202                      |
|         | 5-chloro-2-methyl-4-isothiazolin-3-one/2-methyl-4-isothiazolin-3-one(3/1) | 0.0001                      |
|         | SF-2                                                                      | 0.0032                      |
|         | Tergitol 15-S-5™ (surfactant)                                             | 0.0020                      |
|         | SF-1                                                                      | 0.0081                      |
|         | Aerosol OT™ (surfactant)                                                  | 0.0029                      |

The silver halide imaging layers described above were applied to the polyethylene skin layers of the reflective base using curtain coating. The structure of the photographic element of the example after application of the silver halide imaging layers is as follows:

Silver halide imaging layers  
Biaxially oriented polymer sheet  
Cellulose paper base  
Biaxially oriented polymer sheet  
Silver halide imaging layers

The 10 mm slit rolls of duplitzied light sensitive silver halide reflective material was printed using a digital CRT

photographic printer. The image was printed on one side, the light sensitive image material was then rotated and printed on the opposite side. Several test images were printed on the photographic label material. The printed images were then

5 developed using standard reflective RA4 photographic wet chemistry. After image processing, a 18 micrometer polyester sheet was laminated to both sides of the developed image layers utilizing a acrylic pressure sensitive adhesive. After lamination of the polyester sheet, retaining holes were

10 punched in the image margins for insertion into a photographic album with binder rings.

Oriented polyester

Acrylic pressure sensitive adhesive

Developed silver halide imaging layers

15 Oriented polymer sheet

Cellulose paper

Oriented polymer sheet

Developed imaging layers

Acrylic pressure sensitive adhesive

20 Oriented polyester

The color photographic duplitzied image was superior two sided photographic image compared to prior art two sided images. Because the duplitzied images of the invention utilize one reflective backing material, the amount of reflective base has been reduced by 50% compared to prior art two sides images. Further, because the imaging layers of the invention are protected by a polyester sheet, the imaging layers can better withstand the rigors of consumer handling of the images and insertion into a photographic album.

25 30 Because the imaging materials of the invention are light and thin, they can be mailed at a much lower cost compared to prior art two sided photographic paper which contain a paper core that is twice as thick as the invention.

The photographic elements of the invention also are less 35 susceptible to curl, as the gelatin utilized as a carrier for the silver halide grains and color couplers are sealed from humidity contamination to a great degree. During the image printing step, the voided layers in the top and bottom biaxially oriented sheet in combination with TiO<sub>2</sub> incorpo-

40 rated into the polymer layers provided the required opacity to prevent unwanted exposure of the opposite side. During the printing process, exceptional image sharpness was observed which contributed to the detail and quality of the image. Because the reflective base utilized in the invention

45 contained a high performing biaxially voided oriented polymer sheets containing 24% TiO<sub>2</sub>, the sharpness of the image was improved compared to prior art materials that typically contain 12% TiO<sub>2</sub>.

Finally, because the imaging base of the invention utilized 50 high strength oriented polymer sheets, the tear strength of the photographic album page was 850 N, the need for expensive grommets to prevent fracture around the punched holes was eliminated.

The invention has been described in detail with particular 55 reference to certain preferred embodiments thereof, but it will be understood that variations and modifications can be effected within the spirit and scope of the invention.

What is claimed is:

1. A photographic element comprising a base having a 60 reflection surface on each side having a spectral transmission of less than 10% and at least one photosensitive silver halide containing layer on each side wherein said photographic element has a speed less than 50 ASA.

2. The photographic element of claim 1 wherein said base 65 comprises paper.

3. The photographic element of claim 2 wherein said paper has a water resistant polymer coating on each side.

**55**

- 4. The photographic element of claim 1 wherein said base comprises a voided polyester sheet.
- 5. The photographic element of claim 2 wherein said base comprises a polyester containing white pigment.
- 6. The photographic element of claim 2 wherein said paper is provided with a biaxially oriented polyolefin sheet on each side.
- 7. The photographic element of claim 1 wherein said base contains an opacifying layer.
- 8. The photographic element of claim 1 wherein said base has a light transmission of less than 5%.
- 9. The photographic element of claim 1 wherein said base has a light transmission of less than 2%.
- 10. The photographic element of claim 7 wherein said opacifying layer comprises a metallic layer.
- 11. The photographic element of claim 7 wherein said opacifying layer comprises a polymer layer containing a black pigment or dye.
- 12. The photographic element of claim 1 wherein said base material is free of pin holes.
- 13. The photographic element of claim 1 wherein said element further comprises at least one antihalation layer.
- 14. The photographic element of claim 1 wherein said reflective surfaces have an L star of greater than 93.5.
- 15. The photographic element of claim 1 wherein the outer surface of each side comprises a protective layer comprising gelatin and matte beads.
- 16. The photographic element of claim 1 wherein said element has a stiffness of greater than 100 millinewtons.

**56**

- 17. The photographic element of claim 1 wherein said element has a stiffness of between 100 and 350 millinewtons.
- 18. The photographic element of claim 1 further comprising an antistatic layer between said base and said at least one photosensitive layer on each side of said base.
- 19. A method of forming a duplitized image comprising providing a photographic element comprising a base having a reflection surface on each side having a spectral transmission of less than 10% and at least one photosensitive silver halide containing layer on each side wherein said photographic element has a speed of less than ASA 50, imaging at least one side of said photographic element, and developing said image.
- 20. The method of claim 19 further comprising wherein a first side of said photographic element is imaged, the element is turned over and then the second side is imaged with the same imager.
- 21. The method of claim 19 further comprising punching holes adjacent to at least one edge for placement into an album.
- 22. The method of claim 19 wherein imaging of both sides is carried out substantially simultaneously.
- 23. The method of claim 19 wherein after developing the developed image is covered with a protective polymer.

\* \* \* \* \*